



US008394559B2

(12) **United States Patent**  
**Mitsumori et al.**

(10) **Patent No.:** **US 8,394,559 B2**  
(b5) **Date of Patent:** **Mar. 12, 2013**

(54) **COATING LIQUID FOR FORMING  
UNDERCOAT LAYER, PHOTORECEPTOR  
HAVING UNDERCOAT LAYER FORMED OF  
THE COATING LIQUID, IMAGE-FORMING  
APPARATUS INCLUDING THE  
PHOTORECEPTOR, AND  
ELECTROPHOTOGRAPHIC CARTRIDGE  
INCLUDING THE PHOTORECEPTOR**

(75) Inventors: **Teruyuki Mitsumori**, Yokohama (JP);  
**Shunichiro Kurihara**, Odawara (JP);  
**Hiroe Fuchigami**, Odawara (JP)

(73) Assignee: **Mitsubishi Chemical Corporation**,  
Tokyo (JP)

(\*) Notice: Subject to any disclaimer, the term of this  
patent is extended or adjusted under 35  
U.S.C. 154(b) by 794 days.

(21) Appl. No.: **12/301,376**

(22) PCT Filed: **May 18, 2007**

(86) PCT No.: **PCT/JP2007/060220**

§ 371 (c)(1),  
(2), (4) Date: **Jan. 27, 2009**

(87) PCT Pub. No.: **WO2007/135985**

PCT Pub. Date: **Nov. 29, 2007**

(65) **Prior Publication Data**

US 2009/0232552 A1 Sep. 17, 2009

(30) **Foreign Application Priority Data**

May 19, 2006 (JP) ..... 2006-140863

(51) **Int. Cl.**  
**G03G 5/10** (2006.01)  
**G03G 5/14** (2006.01)

(52) **U.S. Cl.:** **430/57.1; 430/60; 430/65**

(58) **Field of Classification Search:** **430/57.1,  
430/60, 65**  
See application file for complete search history.

(56) **References Cited**

**U.S. PATENT DOCUMENTS**

5,391,448 A 2/1995 Katayama et al.  
(Continued)

**FOREIGN PATENT DOCUMENTS**

|    |           |        |
|----|-----------|--------|
| CN | 1742236 A | 3/2006 |
| JP | 1 176433  | 7/1989 |

(Continued)

**OTHER PUBLICATIONS**

Machine English language translation of JP 2004233678, Aug. 2004.\*

(Continued)

*Primary Examiner* — Hoa V Le

(74) *Attorney, Agent, or Firm* — Oblon, Spivak, McClelland, Maier & Neustadt, L.L.P.

(57) **ABSTRACT**

Provided are a coating liquid for forming an undercoat layer exhibiting high stability, a process for forming the coating liquid, a high-performance electrophotographic photoreceptor that is capable of forming a high-quality image under various use environments and exhibiting reduced image defects such as black spots and color spots, and an image-forming apparatus and electrophotographic cartridge including the electrophotographic photoreceptor. In the coating liquid for forming an undercoat layer of an electrophotographic photoreceptor containing metal oxide particles and a binder resin, the metal oxide particles have a number average particle diameter of 0.10  $\mu\text{m}$  or less and a 10% cumulative particle diameter of 0.060  $\mu\text{m}$  or less which are measured by a dynamic light-scattering method in the coating liquid for forming an undercoat layer.

**17 Claims, 3 Drawing Sheets**



## U.S. PATENT DOCUMENTS

|              |      |         |                      |    |             |         |
|--------------|------|---------|----------------------|----|-------------|---------|
| 5,882,246    | A    | 3/1999  | Inkyo et al.         | JP | 2004 233678 | 8/2004  |
| 5,932,385    | A *  | 8/1999  | Takamura et al. .... | JP | 2005 181467 | 7/2005  |
| 2004/0259009 | A1 * | 12/2004 | Itami et al. ....    | JP | 2005 205681 | 8/2005  |
| 2006/0073400 | A1 * | 4/2006  | Kumano ....          | JP | 2005 292782 | 10/2005 |
| 2006/0088778 | A1   | 4/2006  | Itami et al.         | JP | 2005 331881 | 12/2005 |
| 2006/0134541 | A1   | 6/2006  | Fujii et al.         | JP | 2005 338445 | 12/2005 |
|              |      |         |                      | JP | 2006 58866  | 3/2006  |
|              |      |         |                      | JP | 2006 154753 | 6/2006  |
|              |      |         |                      | WO | 96 39251    | 12/1996 |
|              |      |         |                      | WO | 2006 054397 | 5/2006  |

## FOREIGN PATENT DOCUMENTS

|    |             |         |
|----|-------------|---------|
| JP | 2 275468    | 11/1990 |
| JP | 3 146958    | 6/1991  |
| JP | 6 202366    | 7/1994  |
| JP | 6 273962    | 9/1994  |
| JP | 7 271078    | 10/1995 |
| JP | 10 69116    | 3/1998  |
| JP | 10 260545   | 9/1998  |
| JP | 11 503666   | 3/1999  |
| JP | 11 202519   | 7/1999  |
| JP | 2000 242016 | 9/2000  |
| JP | 2000 258939 | 9/2000  |
| JP | 2001 209200 | 8/2001  |
| JP | 2001 290292 | 10/2001 |
| JP | 2002 311626 | 10/2002 |
| JP | 2003 84472  | 3/2003  |
| JP | 2004 78140  | 3/2004  |
| JP | 2004 233465 | 8/2004  |

## OTHER PUBLICATIONS

U.S. Appl. No. 12/612,982, filed Nov. 5, 2009, Fuchigami.  
 U.S. Appl. No. 12/613,023, filed Nov. 5, 2009, Fuchigami.  
 Office Action issued Mar. 23, 2011, in Chinese Patent Application No. 200780017650.5 (with English-language translation).  
 U.S. Appl. No. 12/301,121, filed Nov. 17, 2008, Mitsumori, et al.  
 U.S. Appl. No. 12/300,943, filed Nov. 14, 2008, Mitsumori, et al.  
 U.S. Appl. No. 12/301,088, filed Nov. 17, 2008, Mitsumori, et al.  
 U.S. Appl. No. 12/301,109, filed Nov. 17, 2008, Mitsumori, et al.  
 U.S. Appl. No. 12/300,853, filed Nov. 14, 2008, Fuchigami, et al.  
 U.S. Appl. No. 12/301,361, filed Nov. 18, 2008, Mitsumori, et al.  
 U.S. Appl. No. 13/188,743, filed Jul. 22, 2011, Fuchigami.

\* cited by examiner

FIG. 1



FIG. 2



FIG. 3



## 1

**COATING LIQUID FOR FORMING  
UNDERCOAT LAYER, PHOTORECEPTOR  
HAVING UNDERCOAT LAYER FORMED OF  
THE COATING LIQUID, IMAGE-FORMING  
APPARATUS INCLUDING THE  
PHOTORECEPTOR, AND  
ELECTROPHOTOGRAPHIC CARTRIDGE  
INCLUDING THE PHOTORECEPTOR**

## TECHNICAL FIELD

The present invention relates to a process for preparing a coating liquid for forming an undercoat layer used for forming an undercoat layer of an electrophotographic photoreceptor by applying and drying the coating liquid, a photoreceptor having a photosensitive layer on the undercoat layer formed of the coating liquid prepared by the process, an image-forming apparatus including the photoreceptor, and an electrophotographic cartridge including the photoreceptor. The electrophotographic photoreceptor including the photosensitive layer on the undercoat layer formed by applying and drying the coating liquid for forming an undercoat layer prepared by the process of the present invention can be suitably applied to, for example, printers, facsimile machines, and copiers of electrophotographic systems.

## BACKGROUND ART

Recently, electrophotographic technology has been widely applied to the field of printers, as well as the field of copiers, due to its immediacy and formation of high-quality images. Photoreceptors lie in the core technology of electrophotography, and organic photoreceptors using organic photoconductive materials have been developed, since they have advantages such as non-pollution and ease in production in comparison with inorganic photoconductive materials. In general, an organic photoreceptor is composed of an electroconductive support and a photosensitive layer disposed thereon. Photoreceptors are classified into a so-called single-layer photoreceptor having a single photosensitive layer containing a binder resin dissolving or dispersing a photoconductive material therein; and a so-called multilayered photoreceptor composed of a plurality of laminated layers including a charge-generating layer containing a charge-generating material and a charge-transporting layer containing a charge-transporting material.

In the organic photoreceptor, changes in use environment of the photoreceptor or changes in electric characteristics during repeated use may cause various defects in an image formed with the photoreceptor. In a reliable method for forming a good image, an undercoat layer containing a binder resin and titanium oxide particles is provided between an electroconductive substrate and a photosensitive layer (for example, refer to Patent Document 1).

The layer of the organic photoreceptor is generally formed by applying and drying a coating liquid prepared by dissolving or dispersing a material in a solvent, because of its high productivity. In such a case, since the titanium oxide particles and the binder resin are incompatible with each other in the undercoat layer, the coating liquid for forming the undercoat layer is provided in the form of a dispersion of titanium oxide particles.

Such a coating liquid has generally been produced by wet-dispersing titanium oxide particles in an organic solvent using a known mechanical pulverizer, such as a ball mill, a sand grind mill, a planetary mill, or a roll mill, by spending a long period of time (for example, refer to Patent Document 1).

## 2

Furthermore, it is disclosed that when titanium oxide particles are dispersed in a coating liquid for forming an undercoat layer using a dispersion medium, an electrophotographic photoreceptor that exhibits excellent characteristics in repeated charging-exposure cycles even under conditions of low temperature and low humidity can be provided using titania or zirconia as the dispersion medium (for example, refer to Patent Document 2). However, since higher-quality images are required, the performance of the conventional technology is insufficient in various respects such as quality of images formed and stability of coating liquids during a manufacturing process.

[Patent Document 1] Japanese Unexamined Patent Application Publication No. HEI 11-202519

[Patent Document 2] Japanese Unexamined Patent Application Publication No. HEI 6-273962

## DISCLOSURE OF INVENTION

## 20 Problems to be Solved by the Invention

The present invention has been made in consideration of the above-described circumstances of the electrophotographic technology, and it is an object to provide a coating liquid for forming an undercoat layer having a high stability, a process for preparing the coating liquid for forming an undercoat layer, an electrophotographic photoreceptor that can form a high-quality image even under various operation conditions and exhibits high performance in forming images that have reduced image defects such as black spots and color spots, and, an image-forming apparatus and an electrophotographic cartridge that include the photoreceptor.

## Means for Solving the Problems

The present inventors have conducted intensive studies for solving the above-mentioned problems and, as a result, have found the fact that an undercoat layer exhibiting high performance can be obtained by controlling the particle size of metal oxide particles contained in a coating liquid for forming an undercoat layer within a specific range; the coating liquid for forming an undercoat layer can particularly exhibit excellent stability during operation, by dispersing the metal oxide particles with a dispersion medium having a diameter smaller than those of dispersion media that are generally used; an electrophotographic photoreceptor including the undercoat layer obtained by applying and drying the coating liquid can exhibit satisfactory electric characteristics even under various operation conditions; and an image-forming apparatus including the photoreceptor can form high-quality images having significantly reduced image defects such as black spots and color spots that are probably caused by dielectric breakdown. The present invention has been thus completed.

Accordingly, a first aspect of the present invention relates to a coating liquid for forming an undercoat layer of an electrophotographic photoreceptor containing metal oxide particles and a binder resin, wherein the metal oxide particles have a number average particle diameter of 0.10  $\mu\text{m}$  or less and a 10% cumulative particle diameter of 0.060  $\mu\text{m}$  or less which are measured by a dynamic light-scattering method in the coating liquid for forming an undercoat layer (Claim 1).

Furthermore, a second aspect of the present invention relates to a process for preparing a coating liquid for forming an undercoat layer of an electrophotographic photoreceptor containing metal oxide particles and a binder resin. The process includes a step of dispersing the metal oxide particles with a medium having an average particle diameter of 5 to 200  $\mu\text{m}$  in a wet agitating ball mill, and the metal oxide particles have a number average particle diameter of 0.10  $\mu\text{m}$  or less and a 10% cumulative particle diameter of 0.060  $\mu\text{m}$  or less

which are measured by a dynamic light-scattering method in the coating liquid for forming an undercoat layer (Claim 2). Preferably, the wet agitating ball mill includes a stator, a slurry-supplying port disposed at one end of the stator, a slurry-discharging port disposed at the other end of the stator, a rotor for agitating and mixing the above-mentioned medium packed in the stator and slurry supplied from the supplying port, and a separator that is rotatably connected to the discharging port and separates the medium and the slurry by centrifugal force to discharge the slurry from the discharging port (Claim 3). The separator of the wet agitating ball mill is connected to the discharging port to rotate in synchronization with the rotor and separates the medium and the slurry by the centrifugal force to discharge the slurry from the discharging port. The separator is preferably of an impeller-type including two disks having blade-fitting grooves on the inner faces facing each other, a blade fitted to the fitting grooves and lying between the disks, and supporting means supporting the disks having the blade therebetween from both sides (Claim 4).

A third aspect of the present invention relates to a process for preparing a coating liquid for forming an undercoat layer of an electrophotographic photoreceptor containing metal oxide particles and a binder resin. The process includes a step of mixing a small particle size dispersion having a number average particle diameter of 0.10  $\mu\text{m}$  or less and a dispersion having a number average particle diameter different from that of the small particle size dispersion which are measured by a dynamic light-scattering method (Claim 5).

A fourth aspect of the present invention relates to a coating liquid for forming an undercoat layer prepared by the process for preparing a coating liquid for forming an undercoat layer of the present invention (Claim 6).

A fifth aspect of the present invention relates to an electrophotographic photoreceptor including an undercoat layer formed by applying and drying the coating liquid for forming an undercoat layer of the present invention (Claim 7). In this electrophotographic photoreceptor, preferably, the undercoat layer has a thickness of 0.1  $\mu\text{m}$  or more and 10  $\mu\text{m}$  or less, and a layer containing a charge-transporting material has a thickness of 5  $\mu\text{m}$  or more and 15  $\mu\text{m}$  or less (Claim 8).

A sixth aspect of the present invention relates to an image-forming apparatus including an electrophotographic photoreceptor, charging means for charging the electrophotographic photoreceptor, image exposure means for forming an electrostatic latent image by subjecting the charged electrophotographic photoreceptor to image exposure, development means for developing the electrostatic latent image with toner, and transfer means for transferring the toner to a transfer object, wherein the photoreceptor is the electrophotographic photoreceptor of the present invention (Claim 9). In this image-forming apparatus, the charging means is preferably in contact with the electrophotographic photoreceptor (Claim 10), and the exposure light used in the image exposure means preferably has a wavelength of 350 nm or more and 600 nm or less (Claim 11).

A seventh aspect of the present invention relates to an electrophotographic cartridge including an electrophotographic photoreceptor and at least one of charging means for charging the electrophotographic photoreceptor and development means for developing an electrostatic latent image formed in the photoreceptor with toner, wherein the photoreceptor is the electrophotographic photoreceptor according to Claim 7 or 8 (Claim 12). This electrophotographic cartridge includes the charging means, and the charging means is preferably in contact with the electrophotographic photoreceptor (Claim 13).

#### Advantages

According to the present invention, the coating liquid for forming an undercoat layer is stabilized without gelation and precipitation of dispersed titanium oxide particles, therefore enabling long storage and use. Furthermore, the coating liquid exhibits reduced changes in physical properties, such as viscosity in use. Consequently, when photosensitive layers are continuously formed on supports by applying and drying the coating liquid, the resulting photosensitive layers can have a uniform thickness. An electrophotographic photoreceptor including an undercoat layer formed with the coating liquid prepared by the process of the present invention exhibits stable electric characteristics even under low temperature and low humidity, thus being excellent in electric characteristics. Accordingly, an image-forming apparatus including the electrophotographic photoreceptor of the present invention can form a satisfactory image having significantly reduced image defects such as black spots and color spots. In particular, an image-forming apparatus in which charging is conducted by charging means arranged in contact with the electrophotographic photoreceptor can form a satisfactory image having significantly reduced image defects such as black spots and color spots. Furthermore, an image-forming apparatus including the electrophotographic photoreceptor of the present invention and using light with a wavelength of 350 nm to 600 nm in the image exposure means exhibits a high initial charging potential and high sensitivity, which can form a high-quality image.

#### BRIEF DESCRIPTION OF DRAWINGS

FIG. 1 is a longitudinal cross-sectional view schematically illustrating a structure of a wet agitating ball mill according to the present invention;

FIG. 2 is a schematic view illustrating the main structure of an embodiment of the image-forming apparatus of the present invention; and

FIG. 3 is an X-ray diffraction spectrum of oxytitanium phthalocyanine used in Examples.

#### REFERENCE NUMERALS

- 1 photoreceptor
- 2 charging device (charging roller)
- 3 exposure device
- 4 development device
- 5 transfer device
- 6 cleaning device
- 7 fixing device
- 41 development bath
- 42 agitator
- 43 supply roller
- 44 development roller
- 45 regulation member
- 71 upper fixing member (fixing roller)
- 72 lower fixing member (fixing roller)
- 73 heating device
- T toner
- P transfer material (paper, medium)
- 14 separator
- 15 shaft
- 16 jacket
- 17 stator
- 19 discharging path
- 21 rotor
- 24 pulley
- 25 rotary joint

- 26 raw slurry supplying port
- 27 screen support
- 28 screen
- 29 product slurry retrieval port
- 31 disk
- 32 blade
- 35 valve element

BEST MODES FOR CARRYING OUT THE  
INVENTION

Embodiments of the present invention will now be described in detail, but the description of components below is merely exemplary embodiments of the present invention. Accordingly, various modifications can be made within the scope of the present invention.

The present invention relates to a coating liquid for forming an undercoat layer of an electrophotographic photoreceptor, a process for preparing the coating liquid, an electrophotographic photoreceptor having an undercoat layer formed of the coating liquid by coating, an image-forming apparatus including the electrophotographic photoreceptor, and an electrophotographic cartridge including the electrophotographic photoreceptor. The electrophotographic photoreceptor according to the present invention includes the undercoat layer and a photosensitive layer on an electroconductive support. The undercoat layer according to the present invention is provided between the electroconductive support and the photosensitive layer and has functions such as an improvement in adhesion between the electroconductive support and the photosensitive layer, covering of blot and scratches of the electroconductive support, prevention of carrier injection due to impurities or non-uniform surface properties, an improvement in uniformity of electric characteristics, prevention of a decrease in surface potential during repeated use, and prevention of a change in local surface potential, which causes image defects. The undercoat layer is unnecessary for achieving photoelectric characteristics.

[I. Coating Liquid for Forming Undercoat Layer]

The coating liquid for forming an undercoat layer of the present invention is used for forming an undercoat layer, and contains metal oxide particles and a binder resin. In addition, the coating liquid for forming an undercoat layer of the present invention generally contains a solvent. Furthermore, the coating liquid for forming an undercoat layer of the present invention may contain other components within the range that do not significantly impair the effects of the present invention.

Furthermore, in the present invention, the coating liquid for forming an undercoat layer is preferably prepared by mixing a small particle size dispersion having a number average particle diameter of 0.10  $\mu\text{m}$  or less and a dispersion having a number average particle diameter different from that of the small particle size dispersion, when the number average particle diameters of the metal oxide particles are measured by a dynamic light-scattering method. The number average diameter of the dispersion having a different number average particle diameter is different from that of the small particle size dispersion by 1% or more. The dispersions to be mixed preferably have a number average particle diameter of 2.0  $\mu\text{m}$  or less in consideration of, for example, dispersion stability, and the diameter is usually 1  $\mu\text{m}$  or less.

The amount of the small particle size dispersion having a number average particle diameter of 0.10  $\mu\text{m}$  or less is preferably 1% or more, more preferably 5% or more, and more preferably 20% or more to the entire dispersion of the metal

oxide particles. The upper limit is not necessarily determined, and, actually, is preferably 99.5% or less.

The coating liquid for forming an undercoat layer prepared by mixing the above-mentioned two or more dispersions preferably has a number average particle diameter of 0.10  $\mu\text{m}$  or less, which is measured by a dynamic light-scattering method, and, more preferably, simultaneously has a 10% cumulative particle diameter of 0.060  $\mu\text{m}$  or less.

Furthermore, the dispersions may be mixed in the form containing or not containing a binder. However, since the dispersion state not containing the binder is unstable, a binder is preferably mixed within 24 hours after the mixing of the dispersions not containing the binder.

[I-1. Metal Oxide Particle]

[I-1-1. Type of Metal Oxide Particles]

Any metal oxide particle that can be used in an electrophotographic photoreceptor can be used as the metal oxide particles contained in the undercoat layer according to the present invention.

Examples of metal oxides that form the metal oxide particles include metal oxides containing single metal elements, such as titanium oxide, aluminum oxide, silicon oxide, zirconium oxide, zinc oxide, and iron oxide; and metal oxides containing multiple metal elements, such as calcium titanate, strontium titanate, and barium titanate. Among them, metal oxide particles composed of a metal oxide having a band gap of 2 to 4 eV are preferred. When the band gap is too small, carrier injection from the electroconductive support easily occurs, resulting in image defects such as black spots and color spots. When the band gap is too large, charge transfer is precluded by electron trapping, resulting in deterioration of electronic characteristics.

Furthermore, the metal oxide particles may be composed of one type of particles or any combination of different types of particles in any ratio. In addition, the metal oxide particles may be composed of one metal oxide or may be any combination of two or more metal oxides in any ratio.

The metal oxide forming the metal oxide particles is preferably titanium oxide, aluminum oxide, silicon oxide, or zinc oxide, more preferably titanium oxide or aluminum oxide, and most preferably titanium oxide.

Furthermore, the metal oxide particles may have any crystal form that does not significantly impair the effects of the present invention. For example, the crystal form of the metal oxide particles composed of titanium oxide (i.e., titanium oxide particles) is not limited and may be any of rutile, anatase, brookite, or amorphous. In addition, these crystal forms of the titanium oxide particles may be present together.

Furthermore, the metal oxide particles may be subjected to various kinds of surface treatment, for example, treatment with a treating agent such as an inorganic material, e.g., tin oxide, aluminum oxide, antimony oxide, zirconium oxide, or silicon oxide or an organic material, e.g., stearic acid, a polyol, or an organic silicon compound.

In particular, when titanium oxide particles are used as the metal oxide particles, surface treatment is preferably conducted with an organic silicon compound. Examples of the organic silicon compound include silicone oils such as dimethylpolysiloxane and methylhydrogenpolysiloxane; organosilanes such as methyltrimethoxysilane and diphenyltrimethoxysilane; silazanes such as hexamethyldisilazane; and silane coupling agents such as vinyltrimethoxysilane,  $\gamma$ -mercaptopropyltrimethoxysilane, and  $\gamma$ -aminopropyltrimethoxysilane.

Furthermore, the metal oxide particles are preferably treated with a silane coupling agent represented by the fol-

lowing Formula (i). The silane coupling agent has high reactivity with metal oxide particles and is therefore favorable.

[Chemical Formula 1]



(i)

In Formula (i), R<sup>1</sup> and R<sup>2</sup> each independently represent an alkyl group. The carbon numbers of R<sup>1</sup> and R<sup>2</sup> are not limited, but are each usually one or more and usually 18 or less, preferably 10 or less, more preferably 6 or less, and most preferably 3 or less. This has an advantage of improved reactivity with metal oxide particles. A larger number of carbon atoms may cause a decrease in the reactivity with metal oxide particles or a decrease in the dispersion stability, in a coating liquid, of the metal oxide particles after treatment.

Preferable examples of R<sup>1</sup> and R<sup>2</sup> include a methyl group, an ethyl group, and a propyl group.

In addition, in Formula (i), R<sup>3</sup> represents an alkyl group or an alkoxy group. The carbon number of R<sup>3</sup> is not limited, but is usually one or more and usually 18 or less, preferably 10 or less, more preferably 6 or less, and most preferably 3 or less. This has an advantage of improved reactivity with metal oxide particles. A larger number of carbon atoms may cause a decrease in the reactivity with metal oxide particles or a decrease in the dispersion stability, in a coating liquid, of the metal oxide particles after treatment.

Preferable examples of R<sup>3</sup> include a methyl group, an ethyl group, a methoxy group, and an ethoxy group. The outermost surfaces of these surface-treated metal oxide particles are usually treated with a treating agent described above. In such a case, the above-described surface treatment may be one type of treatment or may be any combination of two or more types of treatment. For example, before the surface treatment with a silane coupling agent represented by Formula (i), treatment with a treating agent, such as aluminum oxide, silicon oxide, or zirconium oxide, may be conducted. Furthermore, any combination of metal oxide particles subjected to different types of surface treatment in any ratio may be employed.

Examples of commercial products of the metal oxide particles according to the present invention are shown below, but the metal oxide particles according to the present invention are not limited to the products shown below.

Commercially available examples of the titanium oxide particles include ultrafine titanium oxide particles without surface treatment, "TTO-55 (N)"; ultrafine titanium oxide particles coated with Al<sub>2</sub>O<sub>3</sub>, "TTO-55 (A)" and "TTO-55 (B)"; ultrafine titanium oxide particles surface-treated with stearic acid, "TTO-55 (C)"; ultrafine titanium oxide particles surface-treated with Al<sub>2</sub>O<sub>3</sub> and organosiloxane, "TTO-55 (S)"; high-purity titanium oxide "CR-EL"; titanium oxide produced by a sulfate process, "R-550", "R-580", "R-630", "R-670", "R-680", "R-780", "A-100", "A-220", and "W-10"; titanium oxide produced by a chlorine process, "CR-50", "CR-58", "CR-60", "CR-60-2", and "CR-67"; and electro-conductive titanium oxide, "SN-100P", "SN-100D", and "ET-300 W" (these are manufactured by Ishihara Industry Co., Ltd.); titanium oxide such as "R-60", "A-110", and "A-150"; titanium oxide coated with Al<sub>2</sub>O<sub>3</sub>, "SR-1", "R-GL", "R-5N", "R-5N-2", "R-52N", "RK-1", and "A-SP"; titanium oxide coated with SiO<sub>2</sub> and Al<sub>2</sub>O<sub>3</sub>, "R-GX" and "R-7E"; titanium oxide coated with ZnO, SiO<sub>2</sub>, and Al<sub>2</sub>O<sub>3</sub>, "R-650";

and titanium oxide coated with ZrO<sub>2</sub> and Al<sub>2</sub>O<sub>3</sub>, "R-61N" (these are manufactured by Sakai Chemical Industry Co., Ltd.); titanium oxide surface-treated with SiO<sub>2</sub> and Al<sub>2</sub>O<sub>3</sub>, "TR-700"; titanium oxide surface-treated with ZnO, SiO<sub>2</sub>, and Al<sub>2</sub>O<sub>3</sub>, "TR-840" and "TA-500"; titanium oxide without surface treatment, "TA-100", "TA-200", and "TA-300"; and titanium oxide surface-treated with Al<sub>2</sub>O<sub>3</sub>, "TA-400" (these are manufactured by Fuji Titanium Industry Co., Ltd.); and titanium oxide without surface treatment, "MT-150W" and "MT-500B"; titanium oxide surface-treated with SiO<sub>2</sub> and Al<sub>2</sub>O<sub>3</sub>, "MT-100SA" and "MT-500SA"; and titanium oxide surface-treated with SiO<sub>2</sub>, Al<sub>2</sub>O<sub>3</sub> and organosiloxane, "MT-100SAS" and "MT-500SAS" (these are manufactured by Tayca Corp.). Commercially available examples of the aluminum oxide particles include "Aluminium Oxide C" (manufactured by Nippon Aerosil Co., Ltd.).

Commercially available examples of the silicon oxide particles include "200CF" and "R972" (manufactured by Nippon Aerosil Co., Ltd.) and "KEP-30" (manufactured by Nippon Shokubai Co., Ltd.).

Commercially available examples of the tin oxide particles include "SN-100P" (manufactured by Ishihara Industry Co., Ltd.).

Commercially available examples of the zinc oxide particles include "MZ-305S" (manufactured by Tayca Corp.).

#### [I-1-2. Physical Properties of Metal Oxide Particles]

The metal oxide particles according to the present invention satisfy the following requirements for the particle diameter distribution. That is, the metal oxide particles in the coating liquid for forming an undercoat layer of the present invention usually have a number average particle diameter (hereinafter, optionally, referred to as Mp), which is measured by a dynamic light-scattering method, of 0.10 μm or less, preferably 95 nm or less, and more preferably 90 nm or less. The number average particle diameter does not have lower limit, but is generally 20 nm or more. The electrophotographic photoreceptor of the present invention, which satisfies the above-mentioned range, exhibits stable repeated exposure-charge characteristics at low temperature and low humidity, and prevents image defects, such as black spots and color spots, from occurring in the resulting image. Metal oxide particles having a number average particle diameter larger than 0.10 μm accelerate precipitate and a larger change in viscosity in the coating liquid, resulting in irregularity of the thickness and the surface properties of the formed undercoat layer. This may adversely affect the quality of overlying layers (such as a charge-generating layer).

Furthermore, the metal oxide particles usually have a 10% cumulative particle diameter of 0.060 μm or less, preferably 55 nm or less, and more preferably 50 nm or less and preferably 10 nm or more and more preferably 20 nm or more.

In the present invention, the 10% cumulative particle diameter is the particle size at a point of 10% in the cumulative curve, when the particle size distribution of the metal oxide particles is measured by the dynamic light-scattering method and when the cumulative curve of the volume particle size distribution is plotted from the minimum particle size where the total volume of the metal oxide particles is 100%.

In conventional electrophotographic photoreceptors, the undercoat layer may contain huge metal oxide particles that extend across the undercoat layer from one surface to the other. Such huge metal oxide particles may cause a defect in an image formed. Furthermore, in the case using contact-type charging means, charge may migrate from an electroconductive substrate to a photosensitive layer through the metal oxide particles when the photosensitive layer is charged, and thereby the charging cannot be properly achieved. However,

in the electrophotographic photoreceptor of the present invention, since the number average particle diameter and the 10% cumulative particle diameter are very small, the number of metal oxide particles having a large size causing the above-described defect is significantly reduced. As a result, in the electrophotographic photoreceptor of the present invention, occurrence of the defect and improper charging can be prevented, and thereby a high-quality image can be formed.

[I-1-3. Methods for Measuring Particle Size Distribution]

The number average particle diameter ( $M_p$ ) and the 10% cumulative particle diameter ( $D_{10}$ ) of the metal oxide particles according to the present invention are directly measured in a coating liquid for forming an undercoat layer of the present invention by a dynamic light-scattering method. The values obtained by the dynamic light-scattering method are used regardless of the form of the metal oxide particles.

In the dynamic light-scattering method, the particle size distribution is determined by irradiating finely dispersed particles with laser light to detect the scattering (Doppler shift) of light beams having different phases depending on the velocity of the Brownian motion of these particles. The various types of particle diameters of the metal oxide particles in the coating liquid for forming an undercoat layer of the present invention are those when the metal oxide particles are stably dispersed in the coating liquid for forming an undercoat layer and do not present particle diameters of the metal oxide particles in a powder form or a wet cake before the dispersion. Specifically, actual measurements of the number average particle diameter ( $M_p$ ) and the 10% cumulative particle diameter ( $D_{10}$ ) are conducted with a dynamic light-scattering particle size analyzer (MICROTRAC UPA, model: 9340-UPA, manufactured by Nikkiso Co., Ltd., hereinafter abbreviated to UPA) under the conditions shown below. The actual measurement is conducted according to the instruction manual of the particle size analyzer (Nikkiso Co., Ltd., Document No. T15-490A00, revision No. E). The dynamic light-scattering particle size analyzer can also measure a volume average particle diameter (hereinafter, optionally, referred to as  $M_v$ ).

Setting of the Dynamic Light-Scattering Particle Size Analyzer

Upper measurement limit: 5.9978  $\mu\text{m}$

Lower measurement limit: 0.0035  $\mu\text{m}$

Number of channels: 44

Measurement time: 300 sec

Measurement temperature: 25° C.

Particle transparency: absorptive

Particle refractive index: N/A (not available)

Particle shape: non-spherical

Density: 4.20 g/cm<sup>3</sup> (\*)

Dispersion medium: solvent used in the coating liquid for forming an undercoat layer

Refractive index of dispersion medium: refractive index of the solvent used in the coating liquid for forming an undercoat layer

(\*) This density value is applicable to titanium dioxide particles, and, for other particles, values described in the instruction manual are used.

In the present invention, a solvent mixture of methanol and 1-propanol (weight ratio: methanol/1-propanol=7/3, refractive index=1.35) is used as the dispersion medium unless otherwise specified.

If the concentration of the coating liquid for forming an undercoat layer is too high and is outside of the range that a measurement apparatus can measure, the coating liquid for forming an undercoat layer is diluted with a solvent mixture of methanol and 1-propanol (weight ratio: methanol/1-propanol=7/3, refractive index=1.35) such that the resulting con-

centration of the coating liquid for forming an undercoat layer is within the measurable range of the measurement apparatus. For example, in the case of the above-mentioned UPA, the coating liquid for forming an undercoat layer is diluted with a solvent mixture of methanol and 1-propanol into a sample concentration index (SIGNAL LEVEL) within the range from 0.6 to 0.8, which is suitable for measurement.

Since, even if such dilution is conducted, it is believed that the volume particle diameter of the metal oxide particles in the coating liquid for forming an undercoat layer does not vary, the number average particle diameter ( $M_p$ ) and the 10% cumulative particle diameter ( $D_{10}$ ) after the dilution are regarded as the number average particle diameter ( $M_p$ ) and the 10% cumulative particle diameter ( $D_{10}$ ) of the metal oxide particles, measured by the dynamic light-scattering method, in the coating liquid for forming an undercoat layer according to the present invention.

The number average diameter  $M_p$  can be calculated based on the results of the above-mentioned measurement of the particle size distribution of metal oxide particles by the following Expression (A):

[Expression 1]

$$M_p = \frac{\sum (n \cdot d)}{\sum (n)} \quad \text{Expression (A)}$$

The volume average diameter  $M_v$  can be calculated based on the results of the above-mentioned measurement of the particle size distribution of metal oxide particles by the following Expression (B):

[Expression 2]

$$M_v = \frac{\sum (n \cdot v \cdot d)}{\sum (n \cdot v)} \quad \text{Expression (B)}$$

In Expressions (A) and (B),  $n$  represents the number of particles,  $v$  represents the volume of particles, and  $d$  represents the diameter of particles.

[I-1-4. Other Physical Properties]

The metal oxide particles according to the present invention may have any average primary particle diameter that does not significantly impair the effects of the present invention. However, the average primary particle diameter of the metal oxide particles according to the present invention is usually 1 nm or more and preferably 5 nm or more and usually 100 nm or less, preferably 70 nm or less, and most preferably 50 nm or less.

Furthermore, this average primary particle diameter can be determined based on the arithmetic mean value of the diameters of particles that are directly observed by a transmission electron microscope (hereinafter, optionally, referred to as "TEM").

Also, the refractive index of the metal oxide particles according to the present invention does not have any limitation, and those that can be used in electrophotographic photoreceptors can be used. The refractive index of the metal oxide particles according to the present invention is usually 1.3 or more, preferably 1.4 or more, and more preferably 1.5 or more and usually 3.0 or less, preferably 2.9 or less, and more preferably 2.8 or less.

In addition, as the refractive index of metal oxide particles, reference values described in various publications can be used. For example, they are shown in the following Table 1 according to Filler Katsuyo Jiten (Filler Utilization Dictionary, edited by Filler Society of Japan, Taiseisha LTD., 1994).

TABLE 1

|                               | Refractive index |
|-------------------------------|------------------|
| Titanium oxide (rutile)       | 2.76             |
| Lead titanate                 | 2.70             |
| Potassium titanate            | 2.68             |
| Titanium oxide (anatase)      | 2.52             |
| Zirconium oxide               | 2.40             |
| Zinc sulfide                  | 2.37 to 2.43     |
| Zinc oxide                    | 2.01 to 2.03     |
| Magnesium oxide               | 1.64 to 1.74     |
| Barium sulfate (precipitated) | 1.65             |
| Calcium sulfate               | 1.57 to 1.61     |
| Aluminum oxide                | 1.56             |
| Magnesium hydroxide           | 1.54             |
| Calcium carbonate             | 1.57 to 1.60     |
| Quartz glass                  | 1.46             |

The coating liquid for forming an undercoat layer of the present invention can contain the metal oxide particles and the binder resin at any ratio that does not significantly impair the effects of the present invention. However, in the undercoat layer of the present invention, the amount of the metal oxide particles to one part by weight of the binder resin is usually 0.5 part by weight or more, preferably 0.7 part by weight or more, and more preferably 1.0 part by weight or more and usually 4 parts by weight or less, preferably 3.8 parts by weight or less, and more preferably 3.5 parts by weight or less. A smaller ratio of the metal oxide particles to the binder resin may cause unsatisfactory electric characteristics of the resulting electrophotographic photoreceptor, in particular, an increase in the residual potential. A larger ratio of the metal oxide particles to the binder resin may cause noticeable image defects, such as black spots and color spots, in an image formed with the electrophotographic photoreceptor.

[I-1-5. Methods for Measuring Other Physical Properties]

In a dispersion prepared by dispersing the coating liquid for forming an undercoat layer of the present invention in a solvent mixture of methanol and 1-propanol at a weight ratio of 7:3, the difference between the absorbance to light with 400 nm wavelength and the absorbance to light with 1000 nm wavelength is preferably 1.0 (Abs) or less for metal oxide particles with a refractive index of 2.0 or more, and is preferably 0.02 (Abs) or less for metal oxide particles with a refractive index of 2.0 or less.

The light transmittance can be measured by a generally known absorption spectrophotometer. Since the conditions for measuring light transmittance, such as a cell size and sample concentration, vary depending on physical properties, such as particle diameter and refractive index, of metal oxide particles used, the sample concentration is properly adjusted so as not to exceed the detection limit of a detector in a wavelength region (400 nm to 1000 nm in the present invention) to be measured. In general, the concentration of the metal oxide particles in a sample liquid is controlled to 0.0075 wt % to 0.012 wt %.

The cell size (light path length) used for the measurement is 10 mm. Any cell substantially transparent in the range of 400 nm to 1000 nm can be used. Quartz cells are preferably used, and matched cells having the difference in transmittance characteristics between a sample cell and a standard cell within a predetermined range are particularly preferred.

[I-2. Binder Resin]

The coating liquid for forming an undercoat layer of the present invention can contain any binder resin that does not significantly impair the effects of the present invention. In general, a binder resin that can be used is soluble in a solvent such as an organic solvent and is insoluble or hardly soluble in and substantially immiscible with a solvent such as an organic solvent that is used in a coating liquid for forming a photosensitive layer.

Examples of such a binder resin include phenoxy resins, epoxy resins, polyvinylpyrrolidone, polyvinyl alcohol, casein, polyacrylic acid, celluloses, gelatin, starch, polyurethane, polyimide, and polyamide. These resins may be used alone or in the cured form with a curing agent. In particular, polyamide resins such as alcohol-soluble copolymerized polyamides and modified polyamides exhibit favorable dispersibility and coating characteristics, and are preferred.

Examples of the polyamide resin include so-called copolymerized nylons, such as copolymers of 6-nylon, 66-nylon, 610-nylon, 11-nylon, and 12-nylon; and alcohol-soluble nylon resins, such as chemically modified nylons, e.g., N-alkoxymethyl-modified nylon and N-alkoxyethyl-modified nylon. Examples of commercially available products include "CM4000" and "CM8000" (these are manufactured by Toray Industries, Inc.), and "F-30K", "MF-30", and "EF-30T" (these are manufactured by Nagase Chemtex Corporation).

Among these polyamide resins, particularly preferred is a copolymerized polyamide resin containing a diamine component corresponding to a diamine represented by the following Formula (ii) (hereinafter, optionally, referred to as "diamine component corresponding to Formula (ii)").

[Chemical Formula 2]



In Formula (ii), each of R<sup>4</sup> to R<sup>7</sup> represents a hydrogen atom or an organic substituent, and m and n each independently represent an integer of from 0 to 4. When a plurality of the substituents are present, these substituents may be the same or different from each other.

Preferable examples of the organic substituent represented by R<sup>4</sup> to R<sup>7</sup> include hydrocarbon groups that may contain hetero atoms. Among them, preferred examples are alkyl groups such as a methyl group, an ethyl group, an n-propyl group, and an isopropyl group; alkoxy groups such as a methoxy group, an ethoxy group, an n-propoxy group, and an isopropoxy group; and aryl groups such as a phenyl group, a naphthyl group, an anthryl group, and a pyrenyl group. More preferred are an alkyl group and an alkoxy group; and particularly preferred are a methyl group and an ethyl group.

The number of the carbon atoms in the organic substituent represented by R<sup>4</sup> to R<sup>7</sup> is not limited as long as the effects of the present invention are not significantly impaired, and is usually 20 or less, preferably 18 or less, and more preferably 12 or less and usually 1 or more. When the number of the carbon atoms is too large, the solubility to a solvent is decreased. Consequently, the coating liquid gelates, or becomes cloudy or gelates with a lapse of time even if the resin can be temporarily dissolved.

13

The copolymerized polyamide resin containing a diamine component corresponding to Formula (ii) may contain a constitutional unit other than the diamine component corresponding to Formula (ii) (hereinafter, optionally, referred to as "other polyamide constituent" simply). Examples of the other polyamide constituent include lactams such as  $\gamma$ -butyrolactam,  $\epsilon$ -caprolactam, and lauryllactam; dicarboxylic acids such as 1,4-butanedicarboxylic acid, 1,12-dodecanedicarboxylic acid, and 1,20-eicosanedicarboxylic acid; diamines such as 1,4-butanediamine, 1,6-hexamethylenediamine, 1,8-octamethylenediamine, and 1,12-dodecanediamine; and piperazine. Furthermore, the copolymerized polyamide resin may be, for example, a binary, tertiary, or quaternary copolymer of the constituent.

14

constituents is not limited, but is usually 5 mol % or more, preferably 10 mol % or more, and more preferably 15 mol % or more and usually 40 mol % or less and preferably 30 mol % or less. A significantly large amount of the diamine component corresponding to Formula (ii) may lead to poor stability of the coating liquid. A significantly small amount may lead to low stability of the electric characteristics under conditions of high temperature and high humidity against environmental changes.

10 Examples of the copolymerized polyamide resin are shown below. In these examples, the copolymerization ratio represents the feed ratio (molar ratio) of monomers.

[Chemical Formula 3]

<<<Examples of Polyamide >>>

1



2



3



4



5



6



7



When the copolymerized polyamide resin containing the diamine component corresponding to Formula (ii) contains another polyamide constitutional unit, the amount of the diamine component corresponding to Formula (ii) to the total

65 method without particular limitation and is properly produced by usual polycondensation of polyamide. For example, polycondensation such as melt polymerization, solution

## 15

polymerization, or interfacial polymerization can be properly employed. Furthermore, in the polymerization, for example, a monobasic acid such as acetic acid or benzoic acid; or a monoacidic base such as hexylamine or aniline may be contained in a polymerization system as a molecular weight adjuster.

The binder resins may be used alone or in any combination of two or more kinds in any ratio.

Furthermore, the binder resin according to the present invention may have any number average molecular weight without limitation. For example, for a binder resin of copolymerized polyamide, the number average molecular weight of the copolymerized polyamide is usually 10000 or more and preferably 15000 or more and usually 50000 or less and preferably 35000 or less. If the number average molecular weight is too small or too large, the undercoat layer tends to be difficult to maintain the uniformity.

The binder resin may be contained in the coating liquid for forming an undercoat layer of the present invention at any content that does not significantly impair the effects of the present invention, and the content of the binder resin in the coating liquid for forming an undercoat layer of the present invention is usually 0.5 wt % or more and preferably 1 wt % or more and usually 20 wt % or less and preferably 10 wt % or less.

## [I-3. Solvent]

Any solvent can be used as a solvent for the coating liquid for forming an undercoat layer (solvent for the undercoat layer) of the present invention as long as it can dissolve the binder resin according to the present invention. The solvent is usually an organic solvent, and examples thereof include alcohols containing at most five carbon atoms, such as methanol, ethanol, 1-propanol, and 2-propanol; halogenated hydrocarbons such as chloroform, 1,2-dichloroethane, dichloromethane, trichlene, carbon tetrachloride, and 1,2-dichloropropane; nitrogen-containing organic solvents such as dimethylformamide; and aromatic hydrocarbons such as toluene and xylene.

Furthermore, these solvents may be used alone or in any combination of two or more kinds in any ratio. Furthermore, even if a solvent alone cannot dissolve the binder resin according to the present invention, the solvent can be used in the form of a mixture with another solvent (for example, the organic solvents described above) that can dissolve the binder resin as the mixture. In general, a solvent mixture can advantageously reduce unevenness in coating.

In the coating liquid for forming an undercoat layer of the present invention, the ratio of solid components, such as the metal oxide particles and the binder resin, to the solvent varies depending on the method for coating the coating liquid for forming an undercoat layer and may be determined such that uniform coating can be formed in the coating method that is applied.

## [I-4. Other Components]

The coating liquid for forming an undercoat layer of the present invention may contain other components in addition to the metal oxide particles, the binder resin, and the solvent within a range that does not significantly impair the effects of the present invention. For example, the coating liquid for forming an undercoat layer may contain any additive as the other component.

Examples of the additive include thermal stabilizers represented by sodium phosphite, sodium hypophosphite, phosphorous acid, hypophosphorous acid, and hindered phenol; and other polymerization additives. The additives may be used alone or in any combination of two or more kinds in any ratio.

## 16

## [I-5. Advantage of Coating Liquid for Forming an Undercoat Layer]

The coating liquid for forming an undercoat layer of the present invention has high storage stability. There are many measures of storage stability, for example, in the coating liquid for forming an undercoat layer of the present invention, the rate of change in viscosity after storage for 120 days at room temperature compared to that immediately after the production (i.e., the value obtained by dividing a difference between the viscosity after storage for 120 days and the viscosity immediately after the production by the viscosity immediately after the production) is usually 20% or less, preferably 15% or less, and more preferably 10% or less. The viscosity can be measured by a method in accordance with JIS Z 8803 using an E-type viscometer (product name: ED, manufactured by Tokimec Inc.).

Furthermore, the use of the coating liquid for forming an undercoat layer of the present invention enables highly efficient production of electrophotographic photoreceptors with high quality.

## [II. Process for Preparing Coating Liquid for Forming an Undercoat Layer]

The coating liquid for forming an undercoat layer according to the present invention contains metal oxide particles as described above, and the metal oxide particles are present in the form of dispersion in the coating liquid for forming an undercoat layer. Therefore, the process for preparing the coating liquid for forming an undercoat layer of the present invention usually includes a step of dispersing the metal oxide particles. The process of the present invention is applied to this dispersion step, and other steps do not have particular limitation other than the requirements of the present invention.

## [II-1. Dispersion of Metal Oxide Particles]

In the dispersion treatment of metal oxide particles in the present invention, the metal oxide particles are dispersed in a wet agitating ball mill including a stator, a slurry-supplying port disposed at one end of the stator, a slurry-discharging port disposed at the other end of the stator, a rotor for agitating and mixing a medium packed in the stator and slurry supplied from the supplying port, and a separator for separating the medium and the slurry by centrifugal force to discharge the slurry from the discharging port.

Furthermore, a wet agitating ball mill of which at least a part of the portion that comes into contact with the metal oxide particles is made of a ceramic material having a Young's modulus of 150 to 250 GPa is preferred. In the dispersion step, a dispersion medium having an average particle diameter of 5 to 200  $\mu\text{m}$  is preferably used.

In the dispersion step, the metal oxide particles may be dispersed in a solvent (hereinafter, optionally, the solvent used for dispersion is referred to as "dispersion solvent") by wet dispersion. The slurry supplied during the wet dispersion contains at least the metal oxide particles and the dispersion solvent. By this dispersion step, the metal oxide particles according to the present invention are dispersed and can have, as particularly preferable characteristics, a predetermined particle size distribution described above. Furthermore, the dispersion solvent may be that used in the coating liquid for forming an undercoat layer or may be another solvent. However, when a solvent other than the solvent used in the coating liquid for forming an undercoat layer is used as the dispersion solvent, the metal oxide particles after the dispersion and the solvent to be used in the coating liquid for forming an undercoat layer are mixed or subjected to solvent exchange. In such an occasion, it is preferable that the mixing or the solvent exchange be carried out so as to avoid aggregation of the

metal oxide particles in order to maintain the predetermined particle diameter distribution. Among wet dispersion methods, a dispersion using a dispersion medium is particularly preferred.

The wet agitating ball mill used includes a stator, a slurry-supplying port disposed at one end of the stator, a slurry-discharging port disposed at the other end of the stator, a rotor for agitating and mixing a medium packed in the stator and slurry supplied from the supplying port, and a separator for separating the medium and the slurry by centrifugal force to discharge the slurry from the discharging port. Such a wet agitating ball mill does not have any limitation in the shapes and systems of, for example, the stator, the rotor, and the separator. For example, the rotor may have any shape, and, e.g., a flat plate type, a vertical pin type, or a horizontal pin type can be used. In addition, the mill may be either of a vertical type or a horizontal type.

The dispersion may be conducted with one type of dispersion apparatus or with any combination of two or more types.

In the process for preparing the coating liquid for forming an undercoat layer of an electrophotographic photoreceptor of the present invention, a dispersion medium is used during the dispersion step. The dispersion medium has an average particle diameter of usually 5  $\mu\text{m}$  or more and preferably 10  $\mu\text{m}$  or more and usually 200  $\mu\text{m}$  or less and preferably 100  $\mu\text{m}$  or less. A dispersion medium having a smaller particle diameter tends to give a homogeneous dispersion within a shorter period of time. However, a dispersion medium having an excessively small particle diameter has significantly small mass causing small impact force, which may preclude efficient dispersion.

The coating liquid for forming an undercoat layer prepared using the metal oxide particles dispersed in the wet agitating ball mill with the dispersion medium having the above-mentioned average particle diameter sufficiently satisfies the requirements of the coating liquid for forming an undercoat layer according to the present invention.

Furthermore, at least two dispersions to be mixed with each other are preferably prepared by dispersing the metal oxide particles with different dispersion media. The difference in the diameters of the dispersion media is preferably at least 10  $\mu\text{m}$  or more and more preferably 30  $\mu\text{m}$  or more. The upper limit is preferably 20 mm or less, more preferably 10 mm or less, and further preferably 6 mm or less. At least one of the dispersions to be mixed is preferably prepared in the above-mentioned liquid circulating type wet agitating ball mill.

Since the dispersion medium is substantially spherical, the average particle diameter can be determined by a sieving method using sieves described in, for example, JIS Z 8801: 2000 or image analysis, and the density can be measured by Archimedes's method. For example, the average particle diameter and the sphericity of the dispersion medium can be measured with an image analyzer represented by LUZEX50 manufactured by Nireco Corp.

The density of the dispersion medium is not limited, but is usually 5.5 g/cm<sup>3</sup> or more, preferably 5.9 g/cm<sup>3</sup> or more, and more preferably 6.0 g/cm<sup>3</sup> or more. In general, a dispersion medium having a higher density tends to give homogeneous dispersion within a shorter time. The sphericity of the dispersion medium used is preferably 1.08 or less and more preferably 1.07 or less.

As the material of the dispersion medium, any known dispersion medium can be used, as long as it is insoluble in a dispersion solvent contained in the above-mentioned slurry, has a specific gravity higher than that of the slurry, and does not react with the slurry nor decompose the slurry. Examples of the dispersion medium include steel balls such as chrome

balls (bearing steel balls) and carbon balls (carbon steel balls); stainless steel balls; ceramic balls such as silicon nitride, silicon carbide, zirconium, and alumina balls; and balls coated with films of, for example, titanium nitride or titanium carbonitride. Among them, ceramic balls are preferred, and fired zirconium balls are particularly preferred. More specifically, fired zirconium beads described in Japanese Patent No. 3400836 are particularly preferred.

The dispersion media may be used alone or in any combination of two or more kinds in any ratio.

Among the above-mentioned wet agitating ball mills, particularly preferred is a mill including a cylindrical stator. Furthermore, the mill preferably includes an impeller-type separator that is rotatably connected to a discharging port and separates the dispersion medium and the slurry by centrifugal force to discharge the slurry from the discharging port.

In the wet agitating ball mill used in the present invention, in order to improve its wear resistance, at least a part of the portion that is in contact with metal oxide particles during dispersion treatment is preferably made of a ceramic material with a Young's modulus of 150 GPa to 250 GPa. The ceramic material can be any known ceramic material that has a Young's modulus of 150 GPa to 250 GPa. In general, examples of such materials include sintered metal oxides, metal carbides, and metal nitrides. The Young's modulus of the ceramic material in the present invention is measured according to the "testing methods for elastic modulus of fine ceramics" of JIS R 1602-1995, which prescribes tests for measuring elastic modulus of fine ceramics at ambient temperature. The Young's modulus of the ceramic material is not substantially affected by ambient temperature, and, in the present invention, it is measured at 20° C. A ceramic material having a Young's modulus higher than 250 GPa is worn during dispersion of metal oxide particles used in the undercoat layer of the present invention, and the worn ceramic material is undesirably present in the undercoat layer. This may deteriorate electrophotographic photoreceptive characteristics. The Young's modulus varies depending on the composition ratio of the ceramic material and the particle diameter and the particle size distribution of material before sintering and is therefore adjusted properly to the range of 150 GPa to 250 GPa prescribed in the present invention. In general, metastable zirconia doped with 2 to 3 mol % of yttrium oxide and alumina-reinforced zirconia in which metastable zirconia doped with 20 to 30 mol % of aluminum oxide have the Young's modulus in the range of 150 GPa to 250 GPa in many cases.

In the wet agitating ball mill according to the present invention, the stator is a tubular container having a hollow portion inside thereof and is provided with a slurry supplying port at one end and a slurry discharging port at the other end. In addition, the hollow portion of the inside is filled with a dispersion medium so that metal oxide particles in slurry are dispersed by the dispersion medium. Furthermore, the slurry is supplied to the inside of the stator from the supplying port, and the slurry in the stator is discharged from the discharging port to the exterior of the stator.

The rotor is disposed in the interior of the stator and promotes mixing of the dispersion medium and the slurry by agitation. The rotor may be of any type, for example, a pin, disk, or annular type.

Furthermore, the separator separates the dispersion medium and the slurry. This separator is connected to the discharging port of the stator, separates the slurry and the dispersion medium in the stator, and discharges the slurry from the discharging port of the stator to the exterior of the stator.

The separator used here may be of any type, for example, a separator that conducts separation with a screen, a separator that conducts separation by centrifugal force, or a separator utilizing the both, and a rotatable impeller-type separator is preferable. The impeller-type separator separates the dispersion medium and the slurry by centrifugal force generated by the rotation of the impeller.

The separator may be rotated in synchronization with the rotor or independently of the rotor.

Furthermore, the wet agitating ball mill preferably includes a shaft serving as a rotary shaft of the separator. In addition, this shaft is preferably provided with a hollow discharging path communicating with the discharging port, at the center of the shaft. That is, it is preferable that the wet agitating ball mill include at least a cylindrical stator, a slurry supplying port disposed at one end of the stator, a slurry discharging port disposed at the other end of the stator, a rotor agitating and mixing a dispersion medium packed in the stator and slurry supplied from the supplying port, an impeller-type separator that is rotatably connected to the discharging port and separates the dispersion medium and the slurry by centrifugal force to discharge the slurry from the discharging port, and a shaft serving as the rotary shaft of the separator where a hollow discharging path connected to the discharging port is disposed in the center of the shaft.

The discharging path provided to the shaft connects the rotary center of the separator and the discharging port of the stator. Therefore, the slurry separated from the dispersion medium by the separator is transported to the discharging port through the discharging path and is then discharged from the discharging port to the exterior of the stator. The discharging path extends through the center of the shaft. Since the centrifugal force does not work at the center of the shaft, the slurry discharged has no kinetic energy. Consequently, wasteful kinetic energy is not generated, and so excess energy is not consumed.

Such a wet agitating ball mill may be horizontally disposed, but is preferably vertically disposed in order to increase the filling ratio of the dispersion medium. In the vertical installation, the discharging port is preferably disposed at the upper end of the mill. Furthermore, the separator is desirably disposed at a position above the level of the packed dispersion medium.

When the discharging port is disposed at the upper end of the mill, the supplying port is disposed at the bottom of the mill. In this case, more preferably, the supplying port consists of a valve seat and a vertically movable valve element that is fitted to the valve seat and has a V-shape, a trapezoidal shape, or a cone shape so as to be in line contact with the edge of the valve seat. With this, an annular slit can be formed between the edge of the valve seat and the valve element to prevent a dispersion medium from passing through. Therefore, at the supplying port, slurry is supplied without deposition of the dispersion medium. In addition, it is possible to discharge the dispersion medium by spreading the slit by lifting the valve element or to seal the mill by closing the slit by lowering the valve element. Furthermore, since the slit is defined by the valve element and the edge of the valve seat, coarse particles (metal oxide particles) in the slurry are barely caught in and, even if caught, the particles can be readily removed upward or downward. Thus, occlusion hardly occurs.

In addition, coarse particles trapped in the slit can be removed from the slit by vertical vibration of the valve element with vibration means, and occlusion itself of the particles can also be prevented. Furthermore, the vibration of the valve element applies shearing force to the slurry to decrease the viscosity thereof, resulting in an increased amount of

slurry passing through the slit (i.e., the amount of supply). Any means can be used for vibrating the valve element without limitation. For example, in addition to mechanical means such as a vibrator, means of changing the pressure of compressed air that acts on a piston combined with the valve element, such as a reciprocating compressor or an electromagnetic switching valve of switching supply and discharge of compressed air, can be used.

Such a wet agitating ball mill is desirably provided with a screen for separating the dispersion medium and a slurry outlet at the bottom so that the slurry remaining in the wet agitating ball mill can be discharged after the completion of dispersion.

Furthermore, in the case that the wet agitating ball mill is vertically disposed, the shaft is pivoted at the upper end of the stator, an O-ring and a mechanical seal having a mating ring are disposed at a bearing portion bearing the shaft disposed at the upper end of the stator, the bearing portion is provided with an annular groove for fitting the O-ring, and the O-ring is fitted to the annular groove, it is preferable that a tapered cut broadening downward be provided at the lower side of the annular groove. That is, it is preferable that the wet agitating ball mill include a cylindrical vertical stator, a slurry supplying port disposed at the bottom of the stator, a slurry discharging port disposed at the upper end of the stator, a shaft pivoted at the upper end of the stator and rotated by driving means such as a motor, a pin-, disk-, or annular rotor fixed to the shaft and agitating/mixing the dispersion medium packed in the stator and the slurry supplied from the supplying port, a separator disposed near the discharging port and separating the dispersion medium from the slurry, and a mechanical seal disposed at the bearing portion bearing the shaft at the upper end of the stator, and that a tapered cut broadening downward be provided at the lower side of an annular groove for fitting an O-ring being in contact with a mating ring of the mechanical seal.

In this wet agitating ball mill, the mechanical seal is provided at the upper end of the stator above the level of the liquid in the center of the shaft at which the dispersion medium and the slurry substantially do not have kinetic energy. This can significantly reduce intrusion of the dispersion medium and the slurry into a gap between the mating ring of the mechanical seal and the lower side portion of the O-ring fitting groove.

Furthermore, the lower side of the annular groove for fitting the O-ring broadens downward by a cut so that the clearance spreads. Therefore, intrusion of the slurry and the dispersion medium or clogging caused by solidification thereof hardly occurs, and the mating ring smoothly follows the seal ring to maintain the functions of the mechanical seal. In addition, the lower portion of the fitting groove to which the O-ring is fitted has a V-shaped cross-section. Since the entire wall is not thin, the strength is maintained, and the O-ring has high holding ability.

In particular, the separator preferably includes two disks having blade-fitting grooves on the inner faces facing each other, a blade fitted to the fitting grooves and lying between the disks, and supporting means supporting the disks having the blade therebetween from both sides. That is, it is preferable that the wet agitating ball mill include a cylindrical stator, a slurry supplying port disposed at one end of the stator, a slurry discharging port disposed at the other end of the stator, a rotor agitating and mixing the dispersion medium packed in the stator and the slurry supplied from the supplying port, and a rotatable separator provided in the stator, connected to the discharging port, separating the slurry from the dispersion medium by centrifugal force, and discharging the slurry from the discharging port, and that the separator

include two disks having fitting grooves for a blade on the inner faces facing each other, the blade fitted to the fitting grooves and lying between the disks, and supporting means supporting the disks having the blade therebetween from both sides. In such a case, preferably, the supporting means is defined by a shoulder of a shouldered shaft and cylindrical pressing means fitted to the shaft and pressing the disks, and supports the disks having the blade therebetween by pinching them from both sides with the shoulder of the shaft and the pressing means. Such a wet agitating ball mill has advantages that a coating liquid has excellent stability and an image formed with an electrophotographic photoreceptor having an undercoat layer formed by applying this coating liquid has reduced image defects.

The structure of the above-described vertical wet agitating ball mill will now be more specifically described with reference to an embodiment of the wet agitating ball mill. However, the agitating apparatus used for producing the coating liquid for an undercoat layer of the present invention is not limited to those exemplified here.

FIG. 1 is a longitudinal cross-sectional view schematically illustrating a structure of a wet agitating ball mill according to this embodiment. In FIG. 1, slurry (not shown) is supplied to the vertical wet agitating ball mill and is agitated with a dispersion medium (not shown) in the mill for pulverization. Then, the slurry is separated from the dispersion medium by a separator 14 and is discharged through a discharging path 19 in the center of a shaft 15 and then is recycled via a return path (not shown) for further milling.

As shown in FIG. 1 in detail, the vertical wet agitating ball mill has a stator 17 provided with a vertically cylindrical jacket 16 that allows a flow of water for cooling the mill; a shaft 15 that is rotatably born on the upper portion of the stator 17 at the center of the stator 17 and has a mechanical seal at a bearing portion and has a hollow center as a discharging path 19 at the upper portion; pin- or disk-shaped rotors 21 protruding in the radial direction at the lower portion of the shaft 15; a pulley 24, for transmitting driving force, fixed to the upper portion of the shaft 15; a rotary joint 25 mounted on an open end at the upper end of the shaft 15; a separator 14, for separating the medium, fixed to the shaft 15 near the upper portion in the stator 17; a slurry supplying port 26 disposed to the bottom of the stator 17 so as to oppose to the end of the shaft 15; and a screen 28, for separating the dispersion medium, mounted on a grid screen support 27 that is provided to a slurry outlet 29 disposed at an eccentric position of the bottom of the stator 17.

The separator 14 consists of a pair of disks 31 fixed to the shaft 15 with a predetermined interval and a blade 32 connecting these disks 31 to define an impeller and rotates with the shaft 15 to apply centrifugal force to the dispersion medium and the slurry entrapped between the disks 31 for centrifuging the dispersion medium in the radial direction and discharging the slurry through the discharging path 19 in the center of the shaft 15 by the difference in specific gravity.

The slurry supplying port 26 consists of an inverted trap-  
ezoidal valve element 35 that is vertically movable and is fitted to a valve seat disposed at the bottom of the stator 17 and a cylindrical body 36 having a bottom and protruding downward from the bottom of the stator 17. The valve element 35 is lifted upon the supply of slurry to form an annular slit (not shown) with the valve seat, whereby the slurry is supplied to the interior of the stator 17.

When a raw material is supplied, the valve element 35 is lifted by a supply pressure due to the slurry supplied to the inside of the cylindrical body 36, against the pressure in the mill, to form a slit between itself and the valve seat.

In order to prevent clogging of the slit, the valve element 35 repeats vertical shock involving lifting to the upper limit position within a short cycle. This vibration of the valve element 35 may be constantly performed, or may be performed when a large amount of coarse particles are contained in the slurry or in conjunction with an increase in supply pressure of the slurry due to clogging.

An example of the wet agitating ball mill having a structure shown in this embodiment is an Ultra Apex Mill manufactured by Kotobuki Industries Co., Ltd.

Using the wet agitating ball mill of this embodiment having such a structure, slurry is dispersed through the following procedures: A dispersion medium (not shown) is packed in the stator 17 of the wet agitating ball mill of this embodiment, 15 the rotors 21 and the separator 14 are rotated by driving force from an external power source, while a predetermined amount of slurry is supplied from the supplying port 26. As a result, the slurry is supplied to the interior of the stator 7 through the slit (not shown) formed between the edge of the 20 valve seat and the valve element 35.

The slurry and the dispersion medium in the stator 7 are agitated and mixed by the rotation of the rotors 21 to pulverize the slurry. Furthermore, the dispersion medium and the slurry transferred by the rotation of the separator 14 into the separator 14 are separated from each other by the difference in specific gravity. The dispersion medium, which has a larger specific gravity, is centrifuged in the radial direction, and the slurry, which has a smaller specific gravity, is discharged through the discharging path 19 in the center of the shaft 15 toward a raw material tank. When the pulverization proceeds to some extent, the particle size may be optionally measured. If a desired particle size is obtained, the raw material pump is stopped once, and then mill driving is stopped to terminate the pulverization.

When metal oxide particles are dispersed in a wet agitating ball mill, the filling rate of the dispersion medium packed in the wet agitating ball mill is not limited, as long as the metal oxide particles can be dispersed into a predetermined particle size distribution. When metal oxide particles are dispersed in such a vertical wet agitating ball mill described above, the filling rate of the dispersion medium packed in the wet agitating ball mill is usually 50% or more, preferably 70% or more, and more preferably 80% or more and usually 100% or less, preferably 95% or less, and more preferably 90% or less.

The wet agitating ball mill used for dispersing metal oxide particles may have a separator of a screen or slit mechanism, but, as described above, an impeller-type is desirable and a vertical impeller type is preferable. The wet agitating ball mill is desirably of a vertical type having a separator at the upper portion of the mill. In particular, when the filling rate of the dispersion medium is adjusted to the above-mentioned range, pulverization is most efficiently performed, and the separator can be placed at a position higher than the level of the packed medium. This can prevent leakage of a dispersion medium 55 which is carried on the separator.

The operation conditions of the wet agitating ball mill applied to the dispersion of metal oxide particles affect the volume average particle diameter  $M_v$  and the number average particle diameter  $M_p$  of the metal oxide particles in a coating liquid for forming an undercoat layer, the stability of the coating liquid for forming an undercoat layer, the surface shape of the undercoat layer formed by applying the coating liquid, and characteristics of an electrophotographic photoreceptor having the undercoat layer formed by applying the coating liquid for forming an undercoat layer. In particular, the slurry supplying rate and the rotation velocity of the rotor have significant influences.

The slurry-supplying rate affects the residence time of the slurry in the wet agitating ball mill. Accordingly, though the rate varies depending on the capacity and shape of the mill, in the case of a stator usually used, the rate is generally 20 kg/hr or more and preferably 30 kg/hr and usually 80 kg/hr or less and preferably 70 kg/hr or less per liter (hereinafter, optionally, abbreviated to L) of the wet agitating ball mill capacity.

The rotation velocity of the rotor is affected by parameters such as the shape of the rotor or the distance from the stator. In the case of a stator and a rotor usually used, the circumferential velocity at the top end of the rotor is usually 5 m/sec or more, preferably 8 m/sec or more, and more preferably 10 m/sec or more and usually 20 m/sec or less, preferably 15 m/sec or less, and more preferably 12 m/sec or less.

Furthermore, the amount of the dispersion medium is not limited. However, the volume ratio of the dispersion medium to slurry is usually 1 to 5. In the dispersion, a dispersion aid that can be readily removed after the dispersion may be used together with the dispersion medium. Examples of the dispersion aid include sodium chloride and sodium sulfate.

The dispersion of metal oxide particles is preferably carried out by a wet process in the presence of a dispersion solvent. In addition to the dispersion solvent, any additional component may be present as long as the metal oxide particles can be properly dispersed. Examples of such an additional component include a binder resin and various kinds of additives.

Any dispersion solvent can be used without limitation, but the solvent that is used in the coating liquid for forming an undercoat layer is preferably used because of no requirement of steps, such as exchange of solvent, after the dispersion. These dispersion solvents may be used alone or as a solvent mixture of two or more kinds in any combination and any ratio.

The amount of the dispersion solvent used is in the range of usually 0.1 part by weight or more and preferably 1 part by weight or more and usually 500 parts by weight or less and preferably 100 parts by weight or less, on the basis of 1 part by weight of metal oxide particles to be dispersed, from the viewpoint of productivity.

The mechanical dispersion can be carried out at any temperature from the freezing point to the boiling point of a solvent (or solvent mixture), but is usually carried out in the range of 10° C. or higher and 200° C. or lower from the viewpoint of safe manufacturing operation.

After the dispersion treatment using a dispersion medium, it is preferable that the dispersion medium be separated/removed from the slurry and subjected to further sonication. The sonication is a treatment of the metal oxide particles with ultrasonic vibration.

Conditions, such as a vibration frequency, for the sonication are not particularly limited, but ultrasonic vibration with a frequency of usually 10 kHz or more and preferably 15 kHz or more and usually 40 kHz or less and preferably 35 kHz or less from an oscillator is used.

Furthermore, the output of an ultrasonic oscillator is not particularly limited, but is usually 100 W to 5 kW.

In general, dispersion treatment of a small amount of slurry with ultrasound from a low output ultrasonic oscillator is more efficient compared to that of a large amount of slurry with ultrasound from a high output ultrasonic oscillator. Therefore, the amount of slurry to be treated at once is usually 1 L or more, preferably 5 L or more, and more preferably 10 L or more and usually 50 L or less, preferably 30 L or less, and more preferably 20 L or less. The output of an ultrasonic oscillator in such a case is usually 200 W or more, preferably

300 W or more, and more preferably 500 W or more and usually 3 kW or less, preferably 2 kW or less, and more preferably 1.5 kW or less.

The method of applying ultrasonic vibration to metal oxide particles is not particularly limited. For example, the treatment is carried out by directly immersing an ultrasonic oscillator in a container containing slurry, bringing an ultrasonic oscillator into contact with the outer wall of a container containing slurry, or immersing a container containing slurry in a liquid to which vibration is applied with an ultrasonic oscillator. Among these methods, preferably used is the method of immersing a container containing slurry in a liquid to which vibration is applied with an ultrasonic oscillator.

In such a case, the liquid to which vibration is applied with an ultrasonic oscillator is not limited, and examples thereof include water; alcohols such as methanol; aromatic hydrocarbons such as toluene; and oils such as a silicone oil. In particular, water is preferred, in consideration of safe manufacturing operation, cost, washing properties, and other factors.

In the method of immersing the container containing slurry in a liquid to which vibration is applied with an ultrasonic oscillator, since the efficiency of the sonication varies depending on the temperature of the liquid, it is preferable to maintain the temperature of the liquid constant. The applied vibration may raise the temperature of the liquid that is subjected to the ultrasonic vibration. The temperature of the liquid subjected to the sonication is in the range of usually 5° C. or higher, preferably 10° C. or higher, and more preferably 15° C. or higher and usually 60° C. or lower, preferably 50° C. or lower, and more preferably 40° C. or lower.

The container for containing the slurry treated with ultrasound is not limited. For example, any container that is usually used for containing a coating liquid for forming an undercoat layer, which is used for forming a photosensitive layer of an electrophotographic photoreceptor, can be also used. Examples of the container include containers made of resins such as polyethylene or polypropylene, glass containers, and metal cans. Among them, metal cans are preferred. In particular, an 18-liter metal can prescribed in JIS Z 1602 is preferred because of its high resistance to organic solvents and impacts.

The slurry after dispersion or after sonication is filtered before use, according to need, in order to remove coarse particles. The filtration medium in such a case may be any filtering material that is usually used for filtration, such as cellulose fiber, resin fiber, or glass fiber. A preferred form of the filtration medium is a so-called wound filter, which is made of a fiber wound around a core material, because it has a large filtration area to achieve high efficiency. Any known core material can be used, and examples thereof include stainless steel core materials and core materials made of resins, such as polypropylene, that are not dissolved in the slurry and the solvent contained in the slurry.

To the resulting slurry, a solvent, a binder resin (binder), and other optional components (e.g., auxiliary agents) are further added to give a coating liquid for forming an undercoat layer. The metal oxide particles may be mixed with the solvent of the coating liquid for forming an undercoat layer, the binder resin, and the other optional components, in any step of before, during, or after the dispersion or sonication process. Therefore, mixing of the metal oxide particles with the solvent, the binder resin, or the other components may not be necessarily carried out after the dispersion or sonication. [II-2. Advantage in Process for Preparing Coating Liquid for Forming an Undercoat Layer]

The process for preparing a coating liquid for forming an undercoat layer of the present invention enables efficient

preparation of the coating liquid for forming an undercoat layer and also enables the coating liquid for forming an undercoat layer to have higher storage stability. Consequently, an electrophotographic photoreceptor with higher quality is efficiently produced.

[III. Formation of Undercoat Layer]

The undercoat layer according to an electrophotographic photoreceptor can be formed by applying the coating liquid for forming an undercoat layer of the present invention onto an electroconductive support and drying it. The method of applying the coating liquid for forming an undercoat layer of the present invention is not limited, and examples thereof include dip coating, spray coating, nozzle coating, spiral coating, ring coating, bar-coat coating, roll-coat coating, and blade coating. These coating methods may be carried out alone or in any combination of two or more kinds.

Examples of the spray coating include air spray, airless spray, electrostatic air spray, electrostatic airless spray, rotary atomizing electrostatic spray, hot spray, and hot airless spray. In consideration of the fineness of grains for obtaining a uniform thickness and adhesion efficiency, a preferred method is rotary atomizing electrostatic spray disclosed in Japanese Domestic Re-publication (Saikohyo) No. HEI 1-805198, that is, continuous conveyance without spacing in the axial direction with rotation of a cylindrical work. This can give an electrophotographic photoreceptor that exhibits high uniformity of thickness of the undercoat layer with overall high adhesion efficiency.

Examples of the spiral coating method include a method using an injection applicator or a curtain applicator, which is disclosed in Japanese Unexamined Patent Application Publication No. SHO 52-119651; a method of continuously spraying paint in the form of a line from a small opening, which is disclosed in Japanese Unexamined Patent Application Publication No. HEI 1-231966; and a method using a multi-nozzle body, which is disclosed in Japanese Unexamined Patent Application Publication No. HEI 3-193161.

In the case of the dip coating, in general, the total solid content in a coating liquid for forming an undercoat layer is in a range of usually 1 wt % or more and preferably 10 wt % or more and usually 50 wt % or less and preferably 35 wt % or less; and the viscosity is in a range of preferably 0.1 cps or more and preferably 100 cps or less, where 1 cps=1×10<sup>-3</sup> Pa·s.

After the application, the coating is dried. It is preferable that the drying temperature and time be adjusted so as to achieve necessary and sufficient drying. The drying temperature is in a range of usually 100° C. or higher, preferably 110° C. or higher, and more preferably 115° C. or higher and usually 250° C. or lower, preferably 170° C. or lower, and more preferably 140° C. or lower. The drying method is not limited. For example, a hot air dryer, a steam dryer, an infrared dryer, or far-infrared dryer can be used.

[IV. Electrophotographic Photoreceptor]

The electrophotographic photoreceptor of the present invention includes an undercoat layer on an electroconductive support, and a photosensitive layer on the undercoat layer. Therefore, the undercoat layer is disposed between the electroconductive support and the photosensitive layer.

The photosensitive layer can have any composition that can be applied to a known electrophotographic photoreceptor, and examples thereof include a so-called single-layer photoreceptor having a single photosensitive layer (namely, single photosensitive layer) containing a binder resin dissolving or dispersing a photoconductive material therein; and a so-called multilayered photoreceptor composed of a plurality of laminated layers (laminated photosensitive layer) includ-

ing a charge-generating layer containing a charge-generating material and a charge-transporting layer containing a charge-transporting material. It is known that the photoconductive material generally exhibits equivalent functions in both the monolayer and layered photoreceptors.

The photosensitive layer of the electrophotographic photoreceptor of the present invention may be present in any known form, but is preferably a layered photoreceptor, by taking mechanical physical properties, electric characteristics, manufacturing stability, and other characteristics of the photoreceptor into comprehensive consideration. In particular, a normally layered photoreceptor in which an undercoat layer, a charge-generating layer, and a charge-transporting layer are deposited on an electroconductive support in this order is more preferable.

The components of the electrophotographic photoreceptor of the present invention will now be described by the following embodiments, but the components of the electrophotographic photoreceptor of the present invention are not limited to those described in the embodiments below.

[IV-1. Electroconductive Support]

Any electroconductive support can be used without particular limitation, and mainly formed of metal materials such as aluminum, aluminum alloys, stainless steel, copper, and nickel; resin materials provided with conductivity by being mixed with an electroconductive powder, such as a metal, carbon, or tin oxide powder; and resins, glass, and paper on which the surfaces are coated with an electroconductive material, such as aluminum, nickel, or ITO (indium oxide-tin oxide alloy), by vapor deposition or coating.

In addition, the shape of the electroconductive support may be, for example, a drum, a sheet, or a belt. Furthermore, an electroconductive material having an appropriate resistance value may be coated on an electroconductive support of a metal material for controlling conductivity or surface properties or for covering defects.

Furthermore, in the case of the electroconductive support composed of a metal material such as an aluminum alloy, the metal material may be used after anodization treatment. If the anodization treatment is performed, it is desirable to conduct pore sealing treatment by a known method.

For example, an anodic oxide coating is formed by anodization in an acidic bath of, for example, chromic acid, sulfuric acid, oxalic acid, boric acid, or sulfamic acid. Among these acidic baths, anodization in sulfuric acid gives a particularly effective result. In the case of the anodization in sulfuric acid, preferred conditions are a sulfuric acid concentration of 100 to 300 g/L, a dissolved aluminum concentration of 2 to 15 g/L, a liquid temperature of 15 to 30° C., a bath voltage of 10 to 20 V, and a current density of 0.5 to 2 A/dm<sup>2</sup>, but the conditions are not limited thereto.

It is preferable to conduct pore sealing to the resulting anodic oxide coating. The pore sealing may be conducted by a known method and is preferably performed by, for example, low-temperature pore sealing treatment, dipping in an aqueous solution containing nickel fluoride as a main component, or high-temperature pore sealing treatment, dipping in an aqueous solution containing nickel acetate as a main component.

The concentration of the nickel fluoride aqueous solution used in the low-temperature pore sealing treatment may be appropriately determined, but the concentration in the range of 3 to 6 g/L can give a better result. Furthermore, in order to smoothly carry out the pore sealing treatment, the treatment temperature range is usually 25° C. or higher and preferably 30° C. or higher and usually 40° C. or lower and preferably 35° C. or lower. In addition, from the same viewpoint, the pH

range of the nickel fluoride aqueous solution is usually 4.5 or more and preferably 5.5 or more and usually 6.5 or less and preferably 6.0 or less. Examples of a pH regulator include oxalic acid, boric acid, formic acid, acetic acid, sodium hydroxide, sodium acetate, and aqueous ammonia. The treating time is preferably in the range of one to three minutes per micrometer of coating thickness. Furthermore, the nickel fluoride aqueous solution may contain, for example, cobalt fluoride, cobalt acetate, nickel sulfate, or a surfactant in order to further improve the coating physical properties. Then, washing with water and drying complete the low-temperature pore sealing treatment.

On the other hand, examples of the pore sealing agent for the high-temperature pore sealing treatment can include metal salt aqueous solutions of nickel acetate, cobalt acetate, lead acetate, nickel-cobalt acetate, and barium nitrate, and a nickel acetate aqueous solution is particularly preferred. The nickel acetate aqueous solution is preferably used in the concentration range of 5 to 20 g/L. The treatment temperature range is usually 80° C. or higher and preferably 90° C. or higher and usually 100° C. or lower and preferably 98° C. or lower. In addition, the pH of the nickel acetate aqueous solution is preferably in the range of 5.0 to 6.0. Here, examples of the pH regulator can include aqueous ammonia and sodium acetate. The treating time is usually 10 minutes or longer and preferably 15 minutes or longer. Furthermore, the nickel acetate aqueous solution may also contain, for example, sodium acetate, organic carboxylic acid, or an anionic or nonionic surfactant in order to improve physical properties of the coating. In addition, high-temperature water or high-temperature water vapor substantially not containing salts may be used for the treatment. Then, washing with water and drying complete the high-temperature pore sealing treatment.

When the anodic oxide coating has a large average thickness, severer pore sealing conditions may be required for treatment in a higher concentration of pore sealing solution at higher temperature for a longer period of time. In such a case, the productivity is decreased, and also surface defects, such as stains, blot, or blooming, may tend to occur on the coating surface. From these viewpoints, the anodic oxide coating is preferably formed so as to have an average thickness of usually 20  $\mu\text{m}$  or less and particularly preferably 7  $\mu\text{m}$  or less.

The surface of the electroconductive support may be smooth or may be roughened by specific milling or by grinding treatment. In addition, the surface may be roughened by mixing particles having an appropriate particle diameter to the material constituting the support. Furthermore, a drawing tube can be directly used, without conducting milling treatment, for cost reduction. In particular, in the case of use of an aluminum support without milling treatment, such as drawing, impacting, or die processing, blot, adherents such as foreign materials, and small scratches present on the surface are eliminated by the treatment to give a uniform and clean support, and it is therefore preferred.

#### [IV-2. Undercoat Layer]

The undercoat layer contains a binder resin and metal oxide particles. In addition, the undercoat layer may contain other components that do not significantly impair the effects of the present invention. The binder resin, metal oxide particles, and other components are the same as those described in the coating liquid for forming an undercoat layer of the present invention.

Furthermore, in the electrophotographic photoreceptor of the present invention, the number average particle diameter (sic)  $M_p'$  and the 10% cumulative particle diameter  $D_{10}'$  of the metal oxide particles, where these measured by a dynamic light-scattering method in a liquid containing the undercoat

layer dispersed in a solvent mixture of methanol and 1-propanol at a weight ratio of 7:3, satisfy the same requirements as those in the above-described number average particle diameter (sic)  $M_p$  and 10% cumulative particle diameter  $D_{10}$  of the coating liquid for forming an undercoat layer. Accordingly, in the electrophotographic photoreceptor of the present invention, the metal oxide particles preferably have a number average particle diameter  $M_p'$  (sic) of 0.10  $\mu\text{m}$  or less and, simultaneously, preferably have a 10% cumulative particle diameter  $D_{10}'$  of 0.060  $\mu\text{m}$  or less, in a liquid containing the undercoat layer dispersed in a solvent mixture of methanol and 1-propanol at a weight ratio of 7:3.

In the electrophotographic photoreceptor of the present invention, the ratio  $M_p'/M_p$  of a volume average particle diameter  $M_p'$  to a number average diameter  $M_p$  of the metal oxide particles measured by the dynamic light-scattering method in a liquid containing the undercoat layer dispersed in a solvent mixture of methanol and 1-propanol at a weight ratio of 7:3 preferably satisfies the following Expression (3) and more preferably satisfies the following Expression (4).

$$1.10 \leq M_p'/M_p \leq 1.40 \quad (3)$$

$$1.20 \leq M_p'/M_p \leq 1.35 \quad (4)$$

The investigation by the present inventors has revealed that when the above-mentioned ranges are not achieved, the resulting photoreceptor exhibits unstable repeated exposure-charge characteristics at low temperature and low humidity, which may cause image defects, such as black spots and color spots, in the resulting image.

The volume average particle diameter  $M_p'$  and the number average particle diameter  $M_p$  of the metal oxide particles are measured by the dynamic light-scattering method in a dispersion containing the undercoat layer dispersed in a solvent mixture of methanol and 1-propanol at a weight ratio of 7:3 (this functions as a dispersion medium in the measurement of the particle size), not directly measured in the coating liquid for forming an undercoat layer. In this point, the method for measuring the volume average particle diameter  $M_p'$  and the number average particle diameter  $M_p$  is different from that for measuring the above-described volume average particle diameter  $M_p'$  and the number average particle diameter  $M_p$ , but other points are the same (refer to the description of [II-1-3. Methods for measuring particle size distribution] (sic)).

The undercoat layer according to the present invention may be produced by any method without limitation and is generally formed using the above-described coating liquid for forming an undercoat layer of the present invention.

The undercoat layer may have any thickness. However, from the viewpoints of improvements in photoreceptive characteristics of the electrophotographic photoreceptor of the present invention and in coating characteristics, the thickness is usually 0.1  $\mu\text{m}$  or more and preferably 20  $\mu\text{m}$  or less, more preferably 10  $\mu\text{m}$  or less, and most preferably 6  $\mu\text{m}$  or less. With such a thickness, the resulting photoreceptor hardly causes leakage even at a high applied voltage, while exhibiting low residual potential, and exhibits reduced image defects. Furthermore, the undercoat layer may contain additives such as a known antioxidant.

The undercoat layer according to the present invention may have any surface profile, but usually has characteristic in-plane root mean square roughness (RMS), in-plane arithmetic mean roughness (Ra), and in-plane maximum roughness (P-V). These numerical values are obtained by applying the reference lengths of the root mean square height, arithmetic mean height, and maximum height in the specification of JIS B 0601:2001 to a reference plane. The in-plane root

mean square roughness (RMS) represents the root mean square of  $Z(x)$ 's, which are values in the height direction in the reference plane; the in-plane arithmetic mean roughness (Ra) represents the average of the absolute values of  $Z(x)$ 's; and the in-plane maximum roughness (P-V) represents the sum of the maximum height and the maximum depth of  $Z(x)$ .

The in-plane root mean square roughness (RMS) of the undercoat layer according to the present invention is usually 10 nm or more and preferably 20 nm or more and usually 100 nm or less and preferably 50 nm or less. A smaller in-plane root mean square roughness (RMS) may impair the adhesion to an overlying layer such as a photosensitive layer. A larger roughness may decrease the uniformity of the overlying layer such as the photosensitive layer.

The in-plane arithmetic mean roughness (Ra) of the undercoat layer according to the present invention is usually 10 nm or more and preferably 20 nm or more and usually 100 nm or less and preferably 50 nm or less. A smaller in-plane arithmetic mean roughness (Ra) may impair the adhesion to an overlying layer such as a photosensitive layer. A larger roughness may decrease the uniformity of the overlying layer such as the photosensitive layer.

The in-plane maximum roughness (P-V) of the undercoat layer according to the present invention is usually 100 nm or more and preferably 300 nm or more and usually 1000 nm or less and preferably 800 nm or less. A smaller in-plane maximum roughness (P-V) may impair adhesion to an overlying layer such as a photosensitive layer. A larger roughness may decrease the uniformity of the overlying layer such as the photosensitive layer.

The measures (RMS, Ra, P-V) representing the surface profile may be determined with any surface analyzer that can precisely measure irregularities in the reference plane. Particularly, it is preferred to determine these measures by a method of detecting irregularities on the surface of the sample by combining high-precision phase shift detection with counting of the order of interference fringes using an optical interferometer. More specifically, they are preferably measured by an interference fringe addressing method at a wave mode using Micromap manufactured by Ryoka Systems Inc.

A dispersion prepared by dispersing the undercoat layer according to the present invention in a solvent that can dissolve the binder resin binding the undercoat layer shows light transmittance with specific physical properties. The light transmittance of the dispersion can be measured as in the case of measuring the light transmittance of the coating liquid for forming an undercoat layer of the electrophotographic photoreceptor according to the present invention.

The dispersion of the undercoat layer according to the present invention can be prepared by removing layers, such as the photosensitive layer, disposed on the undercoat layer by dissolving the layers in a solvent that can dissolve these layers on the undercoat layer, but not substantially dissolve the binder resin binding the undercoat layer, and then dissolving the binder resin binding the undercoat layer in a solvent to give the dispersion. The solvent that can dissolve the undercoat layer preferably does not have high light absorption in the wavelength region of 400 nm to 1000 nm.

Examples of the solvent that can dissolve the undercoat layer include alcohols such as methanol, ethanol, 1-propanol, and 2-propanol. In particular, methanol, ethanol, and 1-propanol are preferred. These solvents may be used alone or in any combination of two or more kinds in any ratio.

In a dispersion dispersing the undercoat layer according to the present invention in a solvent mixture of methanol and 1-propanol at a weight ratio of 7:3, the difference between the absorbance to light with 400 nm wavelength and the absor-

bance to light with 1000 nm wavelength (absorbance difference) is as follows: For a refractive index of metal oxide particles of 2.0 or more, the absorbance difference is preferably 0.3 (Abs) or less and more preferably 0.2 (Abs) or less.

5 For a refractive index of metal oxide particles of less than 2.0, the absorbance difference is preferably 0.02 (Abs) or less and more preferably 0.01 (Abs) or less.

The absorbance depends on the solid content in a liquid to be measured. Accordingly, in the measurement of light transmittance and absorbance, the concentration of the metal oxide particles dispersed in the dispersion is preferably adjusted to the range of 0.003 wt % to 0.0075 wt %.

10 The regular reflection rate of the undercoat layer according to the present invention usually shows a value specific to the present invention. The regular reflection rate of the undercoat layer according to the present invention means the rate of the regular reflection of an undercoat layer on an electroconductive support to that of the electroconductive support. Since the regular reflection rate of the undercoat layer varies depending on the thickness of the undercoat layer, the reflectance here is 15 defined as that when the thickness of the undercoat layer is 2  $\mu\text{m}$ .

20 In the undercoat layer according to the present invention, for a refractive index of the metal oxide particles contained in the undercoat layer of 2.0 or more, the ratio of the regular reflectance of 480 nm light on the undercoat layer to the regular reflectance of 480 nm light on the electroconductive support is usually 50% or more, where the ratio is converted into that of the undercoat layer with a thickness of 2  $\mu\text{m}$ .

25 On the other hand, for a refractive index of the metal oxide particles contained in the undercoat layer of less than 2.0, the ratio of the regular reflectance of 400 nm light on the undercoat layer to the regular reflectance of 400 nm light on the electroconductive support is usually 50% or more, where the ratio is converted into that of the undercoat layer with a thickness of 2  $\mu\text{m}$ .

30 Here, even if the undercoat layer contains different types of metal oxide particles with refractive indices of 2.0 or more or different kinds of metal oxide particles with refractive indices less than 2.0, the regular reflection rate is preferably in the above-mentioned range. Furthermore, even if the undercoat layer contains both metal oxide particles with a refractive index of 2.0 or more and metal oxide particles with a refractive index less than 2.0, as in the case of the undercoat layer 35 containing metal oxide particles with a refractive index of 2.0 or more, the ratio of the regular reflectance of 480 nm light on the undercoat layer to the regular reflectance of 480 nm light on the electroconductive support is preferably in the above-mentioned range (50% or more), where the regular reflection rate is converted into that of the undercoat layer with a thickness of 2  $\mu\text{m}$ .

40 Hitherto, cases of the undercoat layer having a thickness of 2  $\mu\text{m}$  are described in detail. In the electrophotographic photoreceptor according to the present invention, however, the thickness of the undercoat layer is not limited to 2  $\mu\text{m}$  and may have any thickness. In the case of the undercoat layer 45 having a thickness other than 2  $\mu\text{m}$ , the regular reflection rate can be measured using a coating liquid for forming an undercoat layer that is used for forming the undercoat layer having a thickness other than 2  $\mu\text{m}$  and forming an undercoat layer having a thickness of 2  $\mu\text{m}$  on an electroconductive support equivalent to the electrophotographic photoreceptor and measuring the regular reflection rate of the undercoat layer. Alternatively, the regular reflection rate of the undercoat layer 50 of the electrophotographic photoreceptor is measured, and then the regular reflection rate may be converted into that of an undercoat layer with a thickness of 2  $\mu\text{m}$ .

A conversion process will be described below.

A layer having a small thickness  $dL$  and being perpendicular to the light is supposed for the detection of specific monochromatic light that passes through the undercoat layer, is regularly reflected on the electroconductive support, and then passes again through the undercoat.

A decrease in intensity  $-dI$  of the light that passed through the layer with a small thickness  $dL$  is proportional to the intensity  $I$  before the light passes through the layer and the layer thickness  $dL$ , as is expressed by the equation ( $k$  is a constant) below.

$$-dI = kIdL \quad \text{Equation (C).}$$

Equation (C) can be modified as follows:

$$-dI/I = kdL \quad \text{Equation (D).}$$

By integrating both sides of Equation (D) over the intervals from  $I_0$  to  $I$  and from 0 to  $L$ , respectively, the following equation is obtained. Here,  $I_0$  represents the intensity of the incident light.

$$\log(I_0/I) = -kL \quad \text{Equation (E).}$$

Equation (E) is identical to one called Lambert's law in a solution system and can be applied to measurement of the reflectance in the present invention.

Equation (E) can be modified as follows:

$$I = I_0 \exp(-kL) \quad \text{Equation (F).}$$

The behavior of the incident light before it reaches the surface of an electroconductive support is represented by Equation (F).

The reflectance on the surface of a cylinder is represented by  $R = I_1/I_0$  where  $I_1$  represents the intensity of the reflected light, since the denominator of the regular reflection rate is reflected light of the incident light on the conductive support.

The light that reaches the surface of the electroconductive support in accordance with Equation (F) is regularly reflected after being multiplied by the reflectance  $R$  and then passes through the optical path  $L$  again toward the surface of the undercoat layer. That is, the following expression is obtained:

$$I = I_0 \exp(-kL) \cdot R \cdot \exp(-kL) \quad \text{Equation (G).}$$

$R = I_1/I_0$  is assigned and the equation is further modified to obtain a relationship:

$$I/I_1 = \exp(-2kL) \quad \text{Equation (H).}$$

This is the reflectance of the undercoat layer relative to the reflectance of the electroconductive support and is defined as the regular reflection rate. As described above, in the case of a 2  $\mu\text{m}$  undercoat layer, the to-and-fro optical path length is 4  $\mu\text{m}$ , and the reflectance  $T$  of the undercoat layer on an optional electroconductive support is a function of the thickness  $L$  of the undercoat layer (in this case, the optical path length is 2  $L$ ) and is represented by  $T(L)$ . From Equation (H), the following equation is obtained:

$$T(L) = I/I_1 = \exp(-2kL) \quad \text{Equation (I).}$$

Furthermore, since the value that should be determined is  $T(2)$ ,  $L=2$  is assigned to Equation (I) to obtain:

$$T(2) = I/I_1 = \exp(-4k) \quad \text{Equation (J),}$$

and  $k$  is deleted by Equations (I) and (J) to obtain:

$$T(2) = T(L)^{2L} \quad \text{Equation (K).}$$

That is, at a thickness  $L$  ( $\mu\text{m}$ ) of the undercoat layer, the reflectance  $T(2)$  for an undercoat layer of 2  $\mu\text{m}$  thickness can be estimated with considerable accuracy by measuring the reflectance  $T(L)$  of the undercoat layer. The thickness  $L$  of the

undercoat layer can be measured by any film thickness measuring apparatus such as a roughness meter.

[IV-3. Photosensitive Layer]

[IV-3-1. Charge-Generating Material]

5 The charge-generating material used in the electrophotographic photoreceptor of the present invention can be any conventional material that has been applied to this use. Examples of such a material include azo pigments, phthalocyanine pigments, anthanthrone pigments, quinacridone pigments, cyanine pigments, pyrylium pigments, thiapyrylium pigments, indigo pigments, polycyclic quinone pigments, and squaric acid pigments. Among them, preferred are phthalocyanine pigments and azo pigments. The phthalocyanine pigments can give photoreceptors with high sensitivity to 10 laser light having a relatively long wavelength, and the azo pigments have sufficient sensitivity to white light and laser light having a relatively short wavelength. Thus, these pigments are excellent.

In the present invention, high efficiency is achieved by 20 using the phthalocyanine compounds as a charge-generating material, which is preferable. Examples of the phthalocyanine compounds include metal-free phthalocyanine and phthalocyanines with which metals such as copper, indium, gallium, tin, titanium, zinc, vanadium, silicon, and germanium, or oxides thereof, halides thereof, hydroxides thereof, or alkoxides thereof are coordinated.

Furthermore, the phthalocyanine compounds may have any crystal form, and, preferred are crystal forms with high-sensitivity, e.g., metal-free phthalocyanines of X-type and 30  $\tau$ -type, titanyl phthalocyanine (alias: oxytitanium phthalocyanine) such as A-type (alias:  $\beta$ -type), B-type (alias:  $\alpha$ -type), and D-type (alias: Y-type), vanadyl phthalocyanine, chloroindium phthalocyanine, chlorogallium phthalocyanine such as II-type, hydroxygallium phthalocyanine such as 35 V-type,  $\mu$ -oxo-gallium phthalocyanine dimer such as G-type and I-type, and  $\mu$ -oxo-aluminum phthalocyanine dimer such as II-type. Among these phthalocyanines, particularly preferred are A-type ( $\beta$ -type), B-type ( $\alpha$ -type), and D-type (Y-type) titanyl phthalocyanines, II-type chlorogallium 40 phthalocyanine, V-type hydroxygallium phthalocyanine, and G-type  $\mu$ -oxo-gallium phthalocyanine dimer.

Furthermore, among these phthalocyanine compounds, preferred are oxytitanium phthalocyanine showing a main diffraction peak at a Bragg angle ( $2\theta \pm 0.2^\circ$ ) of  $27.3^\circ$  in an 45 X-ray diffraction spectrum to  $\text{CuK}\alpha$  characteristic X-rays, oxytitanium phthalocyanine showing main diffraction peaks at  $9.3^\circ$ ,  $13.2^\circ$ ,  $26.2^\circ$ , and  $27.1^\circ$ , dihydroxysilicone phthalocyanine showing main diffraction peaks at  $9.2^\circ$ ,  $14.1^\circ$ ,  $15.3^\circ$ ,  $19.7^\circ$ , and  $27.1^\circ$ , dichlorotin phthalocyanine showing main 50 diffraction peaks at  $8.5^\circ$ ,  $12.2^\circ$ ,  $13.8^\circ$ ,  $16.9^\circ$ ,  $22.4^\circ$ ,  $28.4^\circ$ , and  $30.1^\circ$ , hydroxygallium phthalocyanine showing main diffraction peaks at  $7.5^\circ$ ,  $9.9^\circ$ ,  $12.5^\circ$ ,  $16.3^\circ$ ,  $18.6^\circ$ ,  $25.1^\circ$ , and  $28.3^\circ$ , and chlorogallium phthalocyanine showing diffraction peaks at  $7.4^\circ$ ,  $16.6^\circ$ ,  $25.5^\circ$ , and  $28.3^\circ$ . Among them, oxytitanium 55 phthalocyanine showing a main diffraction peak at  $27.3^\circ$  is most preferred, and oxytitanium phthalocyanine showing main diffraction peaks at  $9.5^\circ$ ,  $24.1^\circ$ , and  $27.3^\circ$  is particularly preferred.

The charge-generating materials may be used alone or in any combination of two or more kinds in any ratio. Accordingly, the above-mentioned phthalocyanine compounds may be used alone or in a mixture of two or more kinds or in a mixed crystal state thereof. Here, the mixture or the mixed crystal state of the phthalocyanine compounds may be prepared by mixing respective constituents afterwards or by causing the mixed state in any production or treatment process of the phthalocyanine compounds, such as synthesis,

pigment formation, or crystallization. Examples of such treatment are acid-paste treatment, milling treatment, and solvent treatment. To cause a mixed crystal state, for example, as described in Japanese Unexamined Patent Application Publication No. HEI 10-48859, two different crystals are mixed and are then mechanically milled into an amorphous state, and then the mixture is converted into a specific crystal state by solvent treatment.

In the case using the phthalocyanine compound, a charge-generating material other than the phthalocyanine compound may be simultaneously used. Examples of such a material include azo pigments, perylene pigments, quinacridone pigments, polycyclic quinone pigments, indigo pigments, benzimidazole pigments, pyrylium salts, thiapyrylium salts, and squarium salts.

The charge-generating material is dispersed in a coating liquid for forming a photosensitive layer, and the charge-generating material may be preliminarily pulverized before being dispersed in the coating liquid for forming a photosensitive layer. The pre-pulverization may be carried out with any apparatus, and is usually carried out with, for example, a ball mill or a sand grind mill. The pulverizing medium to be applied to these pulverizers may be any medium that will not be powdered during the pulverization treatment and it can be easily separated after the dispersion treatment. Examples of such a medium include beads and balls of glass, alumina, zirconia, stainless steel, or ceramic. In the pre-pulverization, the charge-generating material is pulverized into a volume average particle diameter of preferably 500  $\mu\text{m}$  or less and more preferably 250  $\mu\text{m}$  or less. The volume average particle diameter of the charge-generating material may be measured by any method that is usually used by those skilled in the art, but is usually measured by a sedimentation method or a centrifugal sedimentation method.

[IV-3-2. Charge-Transporting Material]

Any charge-transporting material can be used. Examples of the charge-transporting material include polymer compounds such as polyvinyl carbazole, polyvinyl pyrene, polyglycidyl carbazole, and polyacenaphthylene; polycyclic aromatic compounds such as pyrene and anthracene; heterocyclic compounds such as indol derivatives, imidazole derivatives, carbazole derivatives, pyrazole derivatives, pyrazoline derivatives, oxadiazole derivatives, oxazole derivatives, and thiadiazole derivatives; hydrazone compounds such as p-diethylaminobenzaldehyde-N,N-diphenylhydrazone and N-methylcarbazole-3-carbaldehyde-N,N-diphenylhydrazone; styryl compounds such as 5-(4-(di-p-tolylamino)benzylidene)-5H-dibenzo(a,d)cycloheptene; triarylamine compounds such as p-tritylamine; benzidine compounds such as N,N,N',N'-tetraphenylbenzidine; butadiene compounds; and triphenylmethane compounds such as di-(p-di-tolylaminophenyl)methane. Among them, preferred are hydrazone derivatives, carbazole derivatives, styryl compounds, butadiene compounds, triarylamine compounds, benzidine compounds, and products produced by bonding some of these compounds. These charge-transporting materials may be used alone or in any combination of two or more kinds in any ratio.

[IV-3-3. Binder Resin for Photosensitive Layer]

The photosensitive layer of the electrophotographic photoreceptor according to the present invention is formed such that a photoconductive material is bound with a binder resin. Any known binder resin used in electrophotographic photoreceptors can be used as the binder resin for a photosensitive layer. Examples of the binder resin for a photosensitive layer include polymethylmethacrylate, polystyrene, polyvinyl acetate, polyacrylic acid esters, polymethacrylic acid esters,

polyesters, polyarylates, polycarbonates, polyester polycarbonates, polyvinyl acetal, polyvinyl acetacetal, polyvinyl propional, polyvinyl butyral, polysulfones, polyimides, phenoxy resins, epoxy resins, urethane resins, silicone resins, cellulose esters, cellulose ethers, vinyl chloride-vinyl acetate copolymers, and vinyl polymers such as polyvinyl chloride; copolymers thereof; and partially cross-linked hardened products thereof. The binder resins for a photosensitive layer may be used alone or in any combination of two or more kinds at any ratio.

[IV-3-4. Layer Containing Charge-Generating Material]  
Multilayered Photoreceptor

In the case that the electrophotographic photoreceptor of the present invention is a so-called multilayered photoreceptor, the layer containing a charge-generating material is usually a charge-generating layer. However, in the multilayered photoreceptor, the charge-transporting layer may contain a charge-generating material as long as the effects of the present invention are not significantly impaired.

The charge-generating material may have any volume average particle diameter, but is usually 1  $\mu\text{m}$  or less and preferably 0.5  $\mu\text{m}$  or less in the case of the multilayered photoreceptor. The volume average particle diameter of the charge-generating material can be measured as in the measurement of the volume average particle diameter of metal oxide particles contained in the undercoat layer in the present invention or can be measured with a known particle size analyzer employing a laser diffraction scattering method or a light-transmission centrifugal sedimentation method.

The thickness of the charge-generating layer is not limited, but is usually 0.1  $\mu\text{m}$  or more and preferably 0.15  $\mu\text{m}$  or more and usually 2  $\mu\text{m}$  or less and preferably 0.8  $\mu\text{m}$  or less.

In the case that the layer containing the charge-generating material is a charge-generating layer, the amount of the charge-generating material used in the charge-generating layer is usually 30 parts by weight or more and preferably 50 parts by weight or more and usually 500 parts by weight or less and preferably 300 parts by weight or less on the basis of 100 parts by weight of the binder resin for a photosensitive layer contained in the charge-generating layer. A smaller amount of the charge-generating material may cause unsatisfactory electric characteristics of the resulting electrophotographic photoreceptor. A larger amount may deteriorate the stability of the coating liquid.

In addition, the charge-generating layer may contain a known plasticizer for improving film-forming characteristics, flexibility, mechanical strength, and other properties, an additive suppressing residual potential, a dispersion aid for improving dispersion stability, a leveling agent for improving the coating characteristics, a surfactant, a silicone oil, a fluorine-based oil, and other additive.

These additives may be used alone or in any combination of two or more kinds in any ratio.

Single-Layer Photoreceptor

In the case that the electrophotographic photoreceptor of the present invention is a so-called single-layer photoreceptor, the charge-generating material is dispersed in a matrix that contains a binder resin and a charge-transporting material for a photosensitive layer as main components with a blending ratio similar to that of the charge-transporting layer described below.

In the case of the single photosensitive layer, the charge-generating material desirably has a sufficiently small particle diameter. Accordingly, the volume average particle diameter of the charge-generating material in the single photosensitive layer is usually 0.5  $\mu\text{m}$  or less and preferably 0.3  $\mu\text{m}$  or less.

The thickness of the single photosensitive layer is not limited, but is usually 5  $\mu\text{m}$  or more and preferably 10  $\mu\text{m}$  or more and usually 50  $\mu\text{m}$  or less and more preferably 45  $\mu\text{m}$  or less. However, in the case that the undercoat layer according to the present invention has a thickness of 6  $\mu\text{m}$  or less, the thickness of the single photosensitive layer is preferably 20  $\mu\text{m}$  or less, more preferably 15  $\mu\text{m}$  or less, and most preferably 10  $\mu\text{m}$  or less. With such a thickness, the resulting photoreceptor hardly causes leakage even at a high applied voltage, while exhibiting low residual potential, and exhibits reduced image defects.

The amount of the charge-generating material dispersed in the photosensitive layer is not limited, but a smaller amount may cause insufficient sensitivity and a larger amount may cause a decrease in charging performance and a decrease in sensitivity. Accordingly, the amount of the charge-generating material in the single photosensitive layer is usually 0.5 wt % or more and preferably 10 wt % or more and usually 50 wt % or less and preferably 45 wt % or less.

In addition, the photosensitive layer of the single-layer photoreceptor also may contain a known plasticizer for improving film-forming characteristics, flexibility, mechanical strength, and other properties, an additive suppressing residual potential, a dispersion aid for improving dispersion stability, a leveling agent for improving the coating characteristics, a surfactant, a silicone oil, a fluorine-based oil, and other additive. These additives may be used alone or in any combination of two or more kinds in any ratio.

[IV-3-5. Layer Containing Charge-Transporting Material]

In the case that the electrophotographic photoreceptor of the present invention is a so-called multilayered photoreceptor, the layer containing a charge-transporting material is usually a charge-transporting layer. The charge-transporting layer may be made of only a resin having a charge-transporting function, but it is preferably made of a binder resin for a photosensitive layer dispersing or dissolving the charge-transporting material.

The charge-transporting layer may have any thickness, but is usually 5  $\mu\text{m}$  or more, preferably 10  $\mu\text{m}$  or more, and more preferably 15  $\mu\text{m}$  or more and usually 60  $\mu\text{m}$  or less, preferably 45  $\mu\text{m}$  or less, and more preferably 27  $\mu\text{m}$  or less. However, when the thickness of the undercoat layer according to the present invention is 6  $\mu\text{m}$  or less, the thickness is preferably 20  $\mu\text{m}$  or less, more preferably 15  $\mu\text{m}$  or less, and most preferably 10  $\mu\text{m}$  or less. With such a thickness, the resulting photoreceptor hardly causes leakage even at a high applied voltage, while exhibiting low residual potential, and exhibits reduced image defects.

In the case that the electrophotographic photoreceptor of the present invention is a so-called single-layer photoreceptor, the single photosensitive layer is made of a binder resin dispersing or dissolving a charge-transporting material as a matrix dispersing the charge-transporting material.

The binder resin used in the layer containing the charge-transporting material may be the above-mentioned binder resins for a photosensitive layer. Among them, examples of the binder resin that is particularly preferred in the layer containing the charge-transporting material include polymethylmethacrylate, polystyrene, vinyl polymers such as polyvinyl chloride, and copolymers thereof; polycarbonates, polyarylates, polyesters, polyester polycarbonates, polysulfones, polyimides, phenoxy resins, epoxy resins, and silicone resins; and partially cross-linked hardened products thereof. These binder resins may be used alone or in any combination of two or more kinds at any ratio.

The ratio of the charge-transporting material to the binder resin in the charge-transporting layer and the single photo-

sensitive layer is not limited as long as the effects of the present invention are not significantly impaired, and the amount of the charge-transporting material is usually 20 parts by weight or more, preferably 30 parts by weight or more, and more preferably 40 parts by weight or more and usually 200 parts by weight or less, preferably 150 parts by weight or less, and more preferably 120 parts by weight or less, on the basis of 100 parts by weight of the binder resin.

In addition, the layer containing the charge-transporting material may optionally contain any additive, for example, an antioxidant such as hindered phenol or hindered amine, an ultraviolet absorber, a sensitizer, a leveling agent, or an electron-attractive compound. These additives may be used alone or in any combination of two or more kinds in any ratio.

[IV-3-6. Other Layers]

The electrophotographic photoreceptor of the present invention may include any other layer, in addition to the undercoat layer and the photosensitive layer.

An example of the other layer may be an outermost layer, for example, a known surface protection layer or overcoat layer having a main component of a thermoplastic or thermosetting polymer.

[IV-3-7. Method for Forming Layer]

Layers other than the undercoat layer of the photoreceptor may be formed by any method without limitation. For example, as in the formation of the undercoat layer with the coating liquid for forming an undercoat layer of the present invention, the layers are formed in series by repeating the coating and drying steps of coating liquids, which are prepared by dissolving or dispersing materials to be contained in each layer (such as a coating liquid for forming a photosensitive layer, a coating liquid for forming a charge-generating layer, or a coating liquid for forming a charge-transporting layer) in a solvent, by a known coating method, such as dip coating, spray coating, or ring coating. In this case, the coating liquid may contain any additive, such as a leveling agent, an antioxidant, or a sensitizer, according to need for improving the coating characteristics.

The solvent used in the coating liquid is not limited, but, in general, an organic solvent is preferably used. Preferable examples of the solvent include alcohols such as methanol, ethanol, 1-propanol, 2-propanol, 1-hexanol, and 1,3-butane-diol; ketones such as acetone, methyl ethyl ketone, methyl isobutyl ketone, and cyclohexanone; ethers such as dioxane, tetrahydrofuran, and ethylene glycol monomethyl ether; ether ketones such as 4-methoxy-4-methyl-2-pentanone; (halo)aromatic hydrocarbons such as benzene, toluene, xylene, and chlorobenzene; esters such as methyl acetate and ethyl acetate; amides such as N,N-dimethylformamide and N,N-dimethylacetamide; and sulfoxides such as dimethyl sulfoxide. Among these solvents, preferably used are alcohols, aromatic hydrocarbons, ethers, and ether ketones, and more preferably used are toluene, xylene, 1-hexanol, 1,3-butanediol, tetrahydrofuran, and 4-methoxy-4-methyl-2-pentanone.

The solvents may be used alone or in any combination of two or more kinds in any ratio. Examples of solvents that are preferably used in combination include ethers, alcohols, amides, sulfoxides, and ether ketones. Among them, preferred are ethers such as 1,2-dimethoxyethane and alcohols such as 1-propanol. In particular, ethers are preferred, from the viewpoints of crystal form stability and dispersion stability of the phthalocyanine when the coating liquid is prepared using oxytitanium phthalocyanine as the charge-generating material.

The amount of the solvent used in the coating liquid is not limited, and may be suitably determined depending on the composition of the coating liquid and the coating process. [IV-3-8. Advantage of Electrophotographic Photoreceptor of the Present Invention]

The electrophotographic photoreceptor of the present invention forms an image with high quality even under various operation conditions. Also, the electrophotographic photoreceptor exhibits excellent duration stability and hardly causes image defects, such as black spots and color spots. Therefore, when the electrophotographic photoreceptor of the present invention is used for forming an image, a high-quality image is formed, with suppressed environmental effect.

In conventional electrophotographic photoreceptors, the undercoat layer contains huge metal oxide particles that extend across the undercoat layer from one surface to the other. Such huge metal oxide particles may cause defects in an image formed. Furthermore, in the case using contact-type charging means, charge may migrate from the electroconductive support to the photosensitive layer through the metal oxide particles when the photosensitive layer is charged, and thereby the charging may be improperly conducted. However, since the electrophotographic photoreceptor of the present invention includes an undercoat layer containing metal oxide particles having a very small average particle diameter and a suitable particle size distribution, occurrence of defects and improper charging are suppressed to enable the formation of a high-quality image.

[V. Image-Forming Apparatus]

Regarding an embodiment of an image-forming apparatus (image-forming apparatus of the present invention) including the electrophotographic photoreceptor of the present invention, the main structure of the apparatus will now be described with reference to FIG. 2. However, the embodiment is not limited to the following description, and various modifications can be conducted within the scope of the present invention.

As shown in FIG. 2, the image-forming apparatus includes an electrophotographic photoreceptor 1, a charging device (charging means) 2, an exposure device (exposure means; image exposure means) 3, a development device (development means) 4, and a transfer device (transfer means) 5. Furthermore, the image-forming apparatus optionally includes a cleaning device (cleaning means) 6 and a fixation device (fixation means) 7.

The photoreceptor 1 of the image-forming apparatus of the present invention is the above-described electrophotographic photoreceptor of the present invention. That is, in the image-forming apparatus of the present invention including an electrophotographic photoreceptor, charging means for charging the electrophotographic photoreceptor, image exposure means for forming an electrostatic latent image by subjecting the charged electrophotographic photoreceptor to image exposure, development means for developing the electrostatic latent image with toner, and transfer means for transferring the toner to a transfer object, the electrophotographic photoreceptor includes an undercoat layer containing metal oxide particles and a binder resin on an electroconductive support, and a photosensitive layer disposed on the undercoat layer; and the volume average particle diameter  $Mv'$  and the number average particle diameter  $Mp'$  of the metal oxide particles, which are measured by a dynamic light-scattering method in a liquid containing the undercoat layer dispersed in a solvent mixture of methanol and 1-propanol at a weight ratio of 7:3, meet the requirements that the  $Mv'$  is 0.1  $\mu\text{m}$  or less and the ratio  $Mv'/Mp'$  satisfies the above-mentioned

Expression (3). The ratio  $Mv'/Mp'$  more preferably satisfies the above-mentioned Expression (4).

The investigation of the present inventors has revealed that when the volume average particle diameter  $Mv'$  and the ratio  $Mv'/Mp'$  do not satisfy the above-mentioned ranges, the resulting photoreceptor exhibits unstable repeated exposure-charge characteristics at low temperature and low humidity. Consequently, image defects, such as black spots and color spots, frequently occur in images formed with the image-forming apparatus of the present invention, which may cause unclear and unstable image formation by the image-forming apparatus.

The electrophotographic photoreceptor 1 is the above-described electrophotographic photoreceptor of the present invention without any additional requirement. FIG. 2 shows, as such an example, a drum photoreceptor having the above-described photosensitive layer on the surface of a cylindrical electroconductive support. Along the outer surface of this electrophotographic photoreceptor 1, a charging device 2, an exposure device 3, a development device 4, a transfer device 5, and a cleaning device 6 are arranged.

The charging device 2 charges the electrophotographic photoreceptor 1 such that the surface of the electrophotographic photoreceptor 1 is uniformly charged to a predetermined potential. It is preferable that the charging device be in contact with the electrophotographic photoreceptor 1 in order to efficiently utilize the effects of the present invention. FIG. 2 shows a roller charging device (charging roller) as an example of the charging device 2, but other charging devices, for example, corona charging devices such as corotron or scorotron and contacting charging devices such as a charging brush, are widely used.

In many cases, the electrophotographic photoreceptor 1 and the charging device 2 are integrated into a cartridge (hereinafter, optionally, referred to as "photoreceptor cartridge") that is detachable from the body of an image-forming apparatus. When the electrophotographic photoreceptor 1 or the charging device 2 are degraded, the photoreceptor cartridge can be replaced with a new one by detaching the used photoreceptor cartridge from the image-forming apparatus body and attaching the new one to the image-forming apparatus body. In addition, in many cases, toner described below is also stored in a toner cartridge detachable from an image-forming apparatus body. When the toner in the toner cartridge is exhausted in use, the toner cartridge can be detached from the image-forming apparatus body, and a new toner cartridge can be attached to the apparatus body. Furthermore, a cartridge including all the electrophotographic photoreceptor 1, the charging device 2, and the toner may be used.

The exposure device 3 may be of any type that can form an electrostatic latent image on a photosensitive surface of the electrophotographic photoreceptor 1 by exposure (image exposure) to the electrophotographic photoreceptor 1, and examples thereof include halogen lamps, fluorescent lamps, lasers such as a semiconductor laser and a He—Ne laser, and LEDs (light-emitting diodes). Furthermore, the exposure may be conducted by a photoreceptor internal exposure system. Any light can be used for the exposure. For example, the exposure may be carried out with monochromatic light having a wavelength of 780 nm; monochromatic light having a slightly shorter wavelength of 600 nm to 700 nm; or monochromatic light having a shorter wavelength of 350 nm to 600 nm. Among them, the exposure is preferably carried out with monochromatic light having a short wavelength of 350 nm to 600 nm and more preferably a wavelength of 380 nm to 500 nm. The development device 4 develops the electrostatic latent image. The development device 4 may be of any type,

and examples thereof include dry development systems such as cascade development, one-component conductive toner development, and two-component magnetic brush development; and wet development systems. The development device 4 shown in FIG. 2 includes a development tank 41, agitators 42, a supply roller 43, a development roller 44, a control member 45, and the development tank 41 containing toner T. In addition, the development device 4 may be provided with an optional refill device (not shown) for refilling the toner T. This refill device can refill the development tank 41 with toner T from a container such as a bottle or a cartridge.

The supply roller 43 is made of, for example, an electro-conductive sponge. The development roller 44 is, for example, a metal roller made of, e.g., iron, stainless steel, aluminum, or nickel or a resin roller made of such a metal roller coated with, e.g., a silicone resin, a urethane resin, or a fluorine resin. The surface of this development roller 44 may be optionally smoothed or roughened.

The development roller 44 is arranged between the electrophotographic photoreceptor 1 and the supply roller 43 and abuts on both the electrophotographic photoreceptor 1 and the supply roller 43. The supply roller 43 and the development roller 44 are rotated by a rotary drive mechanism (not shown). The supply roller 43 carries the toner T stored and supplies it to the development roller 44. The development roller 44 carries the toner T supplied from the supply roller 43 and brings it into contact with the surface of the electrophotographic photoreceptor 1.

The control member 45 is made of, for example, a resin blade of, e.g., a silicone resin or a urethane resin; a metal blade of, e.g., stainless steel, aluminum, copper, brass, or phosphor bronze; or a blade made of such a metal blade coated with a resin. The control member 45 abuts on the development roller 44 and is biased toward the development roller 44 at a predetermined force (a usual blade line pressure is 5 to 500 g/cm) with, for example, a spring. The control member 45 may have an optional function charging the toner T by frictional electrification.

The agitators 42 are each rotated by a rotary drive mechanism and agitate the toner T and transfer it to the supply roller 43. The blade shapes and sizes of the agitators 42 may be different from each other.

The toner T may be of any type, and polymerized toner prepared by suspension polymerization or emulsion polymerization, as well as powder toner, can be used. In the use of the polymerized toner, a small particle diameter of about 4 to 8  $\mu\text{m}$  is particularly preferred, and various shapes of toner may be used from a spherical shape to a non-spherical shape such as a potato-like shape. The polymerized toner exhibits superior charging uniformity and transferring characteristics and, therefore, can be suitably used for forming an image with higher quality.

The transfer device 5 may be of any type, and devices employing, for example, electrostatic transfer such as corona transfer, roller transfer, or belt transfer; pressure transfer; or adhesive transfer can be used. The transfer device 5 includes a transfer charger, a transfer roller, and a transfer belt that are arranged so as to face the electrophotographic photoreceptor 1. The transfer device 5 transfers a toner image formed in the electrophotographic photoreceptor 1 to a transfer material (transfer object, paper, medium) P by a predetermined voltage (transfer voltage) with a polarity opposite to that of the charged potential of the toner T. In the present invention, it is effective that the transfer device 5 be in contact with the photoreceptor via the transfer material.

The cleaning device 6 may be of any type, and examples thereof include a brush cleaner, a magnetic brush cleaner, an

electrostatic brush cleaner, a magnetic roller cleaner, and a blade cleaner. The cleaning device 6 collects remaining toner adhering to the photoreceptor 1 by scraping the remaining toner with a cleaning member. The cleaning device 6 is unnecessary when the amount of toner remaining on the surface of the photoreceptor is small or substantially zero.

The fixation device 7 is composed of an upper fixation member (fixation roller) 71 and a lower fixation member (fixation roller) 72, and the fixation member 71 or 72 is provided with a heating device 73 therein. FIG. 2 shows an example of the heating device 73 provided inside the upper fixation member 71. The upper and lower fixation members 71 and 72 may be known thermal fixation members, for example, a fixation roller in which a pipe of a metal material, such as stainless steel or aluminum, is coated with a silicone rubber, a fixation roller further having a fluorine resin coating, or a fixation sheet. The upper and lower fixation members 71 and 72 may have a structure for supplying a mold-releasing agent, such as a silicone oil, for improving mold release properties or may have a structure for applying a pressure to each other with, for example, a spring.

The toner transferred onto a recording paper P is heated to be melted when passing through between the upper fixation member 71 and the lower fixation member 72 that are heated to a predetermined temperature, and then is fixed on the recording paper P by cooling thereafter.

The fixation device may be of any type, and examples thereof include, in addition to that described here, devices employing a system of heat roller fixation, flash fixation, oven fixation, or pressure fixation.

In the electrophotographic apparatus having a structure described above, an image is recorded as follows: The surface (photosensitive surface) of the photoreceptor 1 is charged to a predetermined potential (for example, -600 V) with the charging device 2. The charging may be conducted by a direct-current voltage or by a direct-current voltage superimposed by an alternating-current voltage.

Subsequently, the charged photosensitive surface of the photoreceptor 1 is exposed with the exposure device 3 depending on the image to be recorded. Thereby, an electrostatic latent image is formed in the photosensitive surface. This electrostatic latent image formed in the photosensitive surface of the photoreceptor 1 is developed by the development device 4.

In the development device 4, the toner T supplied by the supply roller 43 is spread into a thin layer with the control member (developing blade) 45 and, simultaneously, is charged by friction so as to have a predetermined polarity (here, the toner is charged into negative polarity, which is the same as the polarity of the charge potential of the photoreceptor 1). This toner T is held on the development roller 44 and is conveyed and brought into contact with the surface of the photoreceptor 1.

The charged toner T held on the development roller 44 comes into contact with the surface of the photoreceptor 1, so that a toner image corresponding to the electrostatic latent image is formed on the photosensitive surface of the photoreceptor 1. This toner image is transferred to a recording paper P with the transfer device 5. Thereafter, the toner remaining on the photosensitive surface of the photoreceptor 1 without being transferred is removed with the cleaning device 6.

After the transfer of the toner image to the recording paper P, the recording paper P passes through the fixation device 7 to thermally fix the toner image on the recording paper P. Thereby, an image is finally recorded.

The image-forming apparatus may have a structure that can conduct, for example, a charge elimination step, in addition to the above-described structure. The charge elimination step neutralizes the electrophotographic photoreceptor by exposing the electrophotographic photoreceptor with light. Examples of such a device for the charge elimination include fluorescent lamps and LEDs. In many cases, the light used in the charge elimination step has an exposure energy intensity at least 3 times that of the exposure light.

The structure of the image-forming apparatus may be further modified. For example, the image-forming apparatus may have a structure that conducts steps such as a pre-exposure step and a supplementary charging step, that performs offset printing, or that includes a full-color tandem system using different toners.

In the case that a combination of the photoreceptor 1 and the charging device 2 integrated into a cartridge, it is preferable that the cartridge further include the development device 4. Furthermore, a combination of the photoreceptor 1, the charging device 2, the development device 4, and, according to need, one or more of the exposure device 3, the transfer device 5, the cleaning device 6, and the fixation device 7 may be integrated into an integrated cartridge (electrophotographic cartridge) that is detachable from an electrophotographic apparatus such as a copier or a laser beam printer. That is, in the electrophotographic cartridge of the present invention including at least the electrophotographic photoreceptor, the charging means for charging the electrophotographic photoreceptor, and the development means for developing an electrostatic latent image formed in the electrophotographic photoreceptor with toner, the electrophotographic photoreceptor includes an undercoat layer containing metal oxide particles and a binder resin on an electroconductive support, and a photosensitive layer disposed on the undercoat layer; and the volume average particle diameter  $Mv'$  and the number average particle diameter  $Mp'$  of the metal oxide particles, which are measured by a dynamic light-scattering method in a liquid containing the undercoat layer dispersed in a solvent mixture of methanol and 1-propanol at a weight ratio of 7:3, preferably meet the requirements that the  $Mv'$  is 0.1  $\mu\text{m}$  or less and the ratio of the  $Mv'$  and the  $Mp'$ , i.e.,  $Mv'/Mp'$ , satisfies the above-mentioned Expression (3). The ratio  $Mv'/Mp'$  more preferably satisfies the above-mentioned Expression (4). In particular, when the charging means is in contact with the electrophotographic photoreceptor, the effects of the present invention are significantly achieved. Such an arrangement is thus desirable.

The investigation of the present inventors has revealed that when the volume average particle diameter  $Mv'$  and the ratio  $Mv'/Mp'$  do not satisfy the above-mentioned ranges, the resulting photoreceptor exhibits unstable repeated exposure-charge characteristics at low temperature and low humidity. Consequently, image defects, such as black spots and color spots, frequently occur in images formed with an apparatus employing the electrophotographic cartridge of the present invention, which may cause unclear and unstable image formation.

In this case, as in the cartridge described in the above embodiment, for example, even if the electrophotographic photoreceptor 1 or another member is deteriorated, the maintenance of an image-forming apparatus can be readily performed by detaching the electrophotographic cartridge from the image-forming apparatus body and attaching a new electrophotographic cartridge to the image-forming apparatus body.

The image-forming apparatus and the electrophotographic cartridge of the present invention are capable of forming a

high-quality image. In particular, the image-forming apparatus and the electrophotographic cartridge of the present invention hardly cause quality deterioration even if the transfer device 5 is in contact with the photoreceptor via a transfer material, though the quality of an image is readily deteriorated in conventional apparatuses. Thus, the image-forming apparatus and the electrophotographic cartridge according to the present invention are effective.

[VI. Main Advantages of the Present Invention]

According to the present invention, at least one of advantages described below is achieved.

That is, according to the present invention, the coating liquid for forming an undercoat layer is stabilized without gelation and precipitation of dispersed titanium oxide particles, therefore enabling long storage and use. Furthermore, the coating liquid exhibits reduced changes in physical properties, such as viscosity in use. Consequently, when photosensitive layers are continuously formed on supports by applying and drying the coating liquid, the resulting photosensitive layers have a uniform thickness.

Furthermore, an electrophotographic photoreceptor including an undercoat layer formed with the coating liquid prepared by the process for preparing an coating liquid for forming an undercoat layer of the present invention exhibits stable electric characteristics even under low temperature and low humidity, thus having excellent electric characteristics.

Accordingly, an image-forming apparatus including the electrophotographic photoreceptor of the present invention forms a satisfactory image having significantly reduced image defects such as black spots and color spots. In particular, an image-forming apparatus in which charging is conducted by charging means arranged in contact with the electrophotographic photoreceptor forms a satisfactory image having significantly reduced image defects such as black spots and color spots.

Furthermore, an image-forming apparatus including the electrophotographic photoreceptor of the present invention and using light with a wavelength of 350 nm to 600 nm in the image exposure means exhibits a high initial charging potential and high sensitivity, which enables to form a high-quality image.

EXAMPLES

The present invention will now be further specifically described with reference to Examples and Comparative Examples, but is not limited thereto within the scope of the present invention. In the description of Examples, the term "part(s)" means "part(s) by weight" unless otherwise specified.

Example 1

Surface-treated titanium oxide was prepared by mixing 55 rutile titanium oxide having an average primary particle diameter of 40 nm ("TTO55N", manufactured by Ishihara Sangyo Co., Ltd.) and methyltrimethoxysilane ("TSL8117", manufactured by Toshiba Silicone Co., Ltd.) in an amount of 3 wt % on the basis of the amount of the titanium oxide with 60 a Henschel mixer. One kilogram of raw material slurry composed of a mixture of 50 parts of the surface-treated titanium oxide and 120 parts of methanol was subjected to dispersion treatment for 1 hour using zirconia beads with a diameter of about 150  $\mu\text{m}$  (YTZ, manufactured by Nikkato Corp.) as a dispersion medium and an Ultra Apex Mill (model UAM-65, manufactured by Kotobuki Industries Co., Ltd.) having a mill capacity of about 0.15 L under liquid circulation condi-

tions of a rotor peripheral velocity of 10 m/sec and a liquid flow rate of 10 kg/h to give a titanium oxide dispersion.

The titanium oxide dispersion, a solvent mixture of methanol/1-propanol/toluene, and a pelletized polyamide copolymer composed of  $\epsilon$ -caprolactam [compound represented by the following Formula (A)]/bis(4-amino-3-methylcyclohexyl)methane [compound represented by the following Formula (B)]/hexamethylene diamine [compound represented by the following Formula (C)]/decamethylenedicarboxylic acid [compound represented by the following Formula (D)]/octadecamethylenedicarboxylic acid [compound represented by the following Formula (E)] at a molar ratio of 60%/15%/5%/15%/5% were mixed with agitation under heat to dissolve the pelletized polyamide. The resulting solution was subjected to ultrasonic dispersion treatment for 1 hour with an ultrasonic oscillator at an output of 1200 W and then filtered through a PTFE membrane filter with a pore size of 5  $\mu$ m (Mitex LC, manufactured by Advantech Co., Ltd.) to give a coating liquid A for forming an undercoat layer wherein the weight ratio of the surface-treated titanium oxide/copolymerized polyamide was 3/1, the weight ratio of methanol/1-propanol/toluene in the solvent mixture was 7/1/2, and the solid content was 18.0 wt %.

[Chemical Formula 4]



Regarding the coating liquid A for forming an undercoat layer, the rate of change in viscosity after storage for 120 days at room temperature compared to that immediately after the production (i.e., the value obtained by dividing a difference between the viscosity after storage for 120 days and the viscosity immediately after the production by the viscosity immediately after the production) and the particle size distribution of the titanium oxide particles immediately after the production were measured. The viscosity was measured by a method in accordance with JIS Z 8803 using an E-type viscometer (product name: ED, manufactured by Tokimec Inc.), and the particle size distribution was measured with the UPA. The results are shown in Table 2.

#### Example 2

A coating liquid B for forming an undercoat layer was prepared as in Example 1 except that the dispersion medium

used for dispersion in the Ultra Apex Mill was zirconia beads having a diameter of about 50  $\mu$ m (YTZ, manufactured by Nikkato Corp.), and the physical properties thereof were measured as in Example 1. The results are shown in Table 2.

Furthermore, the coating liquid B for forming an undercoat layer was diluted with a solvent mixture of methanol and 1-propanol=7/3 (weight ratio) such that the solid content was 0.015 wt % (metal oxide particle concentration: 0.011 wt %), and the difference between absorbance to light with 400 nm wavelength and the absorbance to light with 1000 nm wavelength of the diluted coating liquid was measured with a UV-visible spectrophotometer (UV-1650PC, manufactured by Shimadzu Corp.). The results are shown in Table 3.

15

#### Example 3

A coating liquid C for forming an undercoat layer was prepared as in Example 2 except that the rotor peripheral velocity of the Ultra Apex Mill was 12 m/sec, and physical properties thereof were measured as in Example 1. The results are shown in Table 2.

20

#### Example 4

A coating liquid D for forming an undercoat layer was prepared as in Example 3 except that the dispersion medium used for dispersion in the Ultra Apex Mill was zirconia beads having a diameter of about 30  $\mu$ m (YTZ, manufactured by Nikkato Corp.), and the physical properties thereof were measured as in Example 1. The results are shown in Table 2.

25

#### Example 5

A coating liquid E for forming an undercoat layer was prepared as in Example 2 except that the weight ratio of surface-treated titanium oxide/copolymerized polyamide was 2/1, and the difference between absorbance to light with 400 nm wavelength and the absorbance to light with 1000 nm wavelength of the coating liquid E was measured as in Example 2 except that the solid content was 0.015 wt % (metal oxide particle concentration: 0.01 wt %). The results are shown in Table 3.

30

35

40

45

#### Example 6

A coating liquid F for forming an undercoat layer was prepared as in Example 2 except that the weight ratio of surface-treated titanium oxide/copolymerized polyamide was 4/1, and the difference between absorbance to light with 400 nm wavelength and the absorbance to light with 1000 nm wavelength of the coating liquid E was measured as in Example 2 except that the solid content was 0.015 wt % (metal oxide particle concentration: 0.012 wt %). The results are shown in Table 3.

50

55

#### Example 7

A coating liquid G for forming an undercoat layer was prepared as in Example 2 except that aluminum oxide particles having an average primary particle diameter of 13 nm (Aluminum Oxide C, manufactured by Nippon Aerosil Co., Ltd.) were used instead of the surface-treated titanium oxide used in Example 1, the solid content contained was 8.0 wt %, and the weight ratio of aluminum oxide particle/copolymerized polyamide was 1/1. The physical properties of the coating liquid G for forming an undercoat layer were measured as in Example 1. The results are shown in Table 2. The difference

60

65

45

between absorbance to light with 400 nm wavelength and the absorbance to light with 1000 nm wavelength of the coating liquid G was measured as in Example 2 except that the coating liquid G was diluted such that the solid content was 0.015 wt % (metal oxide particle concentration: 0.0075 wt %). The results are shown in Table 3.

#### Comparative Example 1

A coating liquid H for forming an undercoat layer was prepared as in Example 1 except that a dispersion slurry liquid prepared by mixing 50 parts of surface-treated titanium oxide and 120 parts of methanol and dispersing the mixture using alumina balls with a diameter of about 3 mm (HD, manufactured by Nikkato Corp.) for 5 hours was directly used without conducting the step of dispersion using the Ultra Apex Mill. The physical properties were measured as in Examples 1 and 2 except that the solid content was 0.015 wt % (metal oxide particle concentration: 0.011 wt %). The results are shown in Tables 2 and 3.

#### Comparative Example 2

A coating liquid I for forming an undercoat layer was prepared as in Comparative Example 1 except that zirconia balls with a diameter of about 3 mm (YTZ, manufactured by Nikkato Corp.) were used for ball mill dispersion in Comparative Example 1. The physical properties were measured as in Example 1. The results are shown in Table 2.

#### Comparative Example 3

A coating liquid J for forming an undercoat layer was prepared as in Comparative Example 1 except that the weight ratio of surface-treated titanium oxide/copolymerized polyamide was 2/1, and the difference between absorbance to light with 400 nm wavelength and the absorbance to light with 1000 nm wavelength of the coating liquid J was measured as in Example 2 except that the solid content was 0.015 wt % (metal oxide particle concentration: 0.01 wt %). The results are shown in Table 3.

#### Comparative Example 4

A coating liquid K for forming an undercoat layer was prepared as in Comparative Example 1 except that the weight ratio of surface-treated titanium oxide/copolymerized polyamide was 4/1, and the difference between absorbance to light with 400 nm wavelength and the absorbance to light with 1000 nm wavelength of the coating liquid K was measured as in Example 2 except that the solid content was 0.015 wt % (metal oxide particle concentration: 0.012 wt %). The results are shown in Table 3.

#### Example 8A

The coating liquid A for forming an undercoat layer prepared in Example 1 and the coating liquid H for forming an undercoat layer prepared in Comparative Example 1 were mixed at a ratio of 3:1. The resulting mixture was subjected to ultrasonic dispersion treatment for 1 hour with an ultrasonic oscillator at a frequency of 25 kHz and an output of 1200 W to prepare a coating liquid 3AH for forming an undercoat layer, and the physical properties were measured as in Example 1. The results are shown in Table 2.

#### Example 8B

The coating liquid A for forming an undercoat layer prepared in Example 1 and the coating liquid H for forming an

46

undercoat layer prepared in Comparative Example 1 were mixed at a ratio of 1:1. The resulting mixture was subjected to ultrasonic dispersion treatment for 1 hour with an ultrasonic oscillator at a frequency of 25 kHz and an output of 1200 W to prepare a coating liquid AH for forming an undercoat layer, and the physical properties were measured as in Example 1. The results are shown in Table 2.

#### Example 8C

The coating liquid A for forming an undercoat layer prepared in Example 1 and the coating liquid H for forming an undercoat layer prepared in Comparative Example 1 were mixed at a ratio of 1:3. The resulting mixture was subjected to ultrasonic dispersion treatment for 1 hour with an ultrasonic oscillator at a frequency of 25 kHz and an output of 1200 W to prepare a coating liquid A3H for forming an undercoat layer, and the physical properties were measured as in Example 1. The results are shown in Table 2.

#### Comparative Example 5

A coating liquid N for forming an undercoat layer was prepared as in Comparative Example 1 except that Aluminum Oxide C (aluminum oxide particles) having an average primary particle diameter of 13 nm, manufactured by Nippon Aerosil Co., Ltd., was used instead of the surface-treated titanium oxide used in Comparative Example 1, the solid content contained was 8.0 wt %, the weight ratio of aluminum oxide particle/copolymerized polyamide was 1/1, and dispersion was conducted for 6 hours with an ultrasonic oscillator at an output of 600 W instead of the ball mill. The physical properties of the coating liquid N for forming an undercoat layer were measured as in Example 1. The results are shown in Table 2. The difference between absorbance to light with 400 nm wavelength and the absorbance to light with 1000 nm wavelength of the coating liquid N was measured as in Example 2 except that the solid content was 0.015 wt % (metal oxide particle concentration: 0.0075 wt %). The results are shown in Table 3.

#### [Evaluation of Regular Reflection Rate]

The regular reflection rate of each of the undercoat layers formed on electroconductive supports with the coating liquids for forming an undercoat layer prepared in Examples and Comparative Examples were evaluated as follows. The results are shown in Table 4.

Undercoat layers with a dried thickness of 2  $\mu\text{m}$  were each formed by applying the coating liquid for forming an undercoat layer shown in Table 4 to an aluminum tube (an extruded mirror surface tube or a cut tube) having an outer diameter of 30 mm, a length of 250 mm, and a thickness of 0.8 mm and drying the liquid.

The reflectance of the undercoat layer to light of 400 nm or light of 480 nm was measured with a multispectrophotometer (MCPD-3000, manufactured by Otsuka Electronics Co., Ltd.). A halogen lamp was used as a light source, and the light source and the tip of a fiber-optic cable mounted on a detector were arranged at a position apart from the surface of the undercoat layer by 2 mm in the vertical direction. The surface of the undercoat layer was irradiated with light from the direction perpendicular to the surface, and reflected light in the opposite direction on the same axis was detected. The light reflected from the surface of a cut aluminum tube without the undercoat layer was measured, and this reflectance was defined as 100%. The light reflected from the surface of the undercoat layer was measured, and the ratio of this value to the above value was defined as regular reflection rate (%).

TABLE 2

| Physical properties of coating liquid for forming an undercoat layer |                |          |                 |                           |                             |          |         |
|----------------------------------------------------------------------|----------------|----------|-----------------|---------------------------|-----------------------------|----------|---------|
|                                                                      | Coating liquid | Medium   | Medium diameter | Rotor peripheral velocity | Rate of change in viscosity | D10 (μm) | Mp (μm) |
| Example 1                                                            | A              | zirconia | 150 μm          | 10 m/s                    | 2% increase                 | 0.0515   | 0.0874  |
| Example 2                                                            | B              | zirconia | 50 μm           | 10 m/s                    | 4% increase                 | 0.0481   | 0.0634  |
| Example 3                                                            | C              | zirconia | 50 μm           | 12 m/s                    | 3% increase                 | 0.0448   | 0.0632  |
| Example 4                                                            | D              | zirconia | 30 μm           | 12 m/s                    | 2% increase                 | 0.0432   | 0.0592  |
| Example 7                                                            | G              | zirconia | 150 μm          | 10 m/s                    | —                           | 0.0524   | 0.0624  |
| Example 8A                                                           | 3AH            | zirconia | 150 μm          | 10 m/s                    | 3% increase                 | 0.0581   | 0.0862  |
|                                                                      |                | alumina  | 3 mm            |                           |                             |          |         |
| Example 8B                                                           | AH             | zirconia | 150 μm          | —                         | 2% increase                 | 0.0504   | 0.0914  |
|                                                                      |                | alumina  | 3 mm            |                           |                             |          |         |
| Example 8C                                                           | A3H            | zirconia | 150 μm          | 10 m/s                    | 4% increase                 | 0.0585   | 0.0960  |
|                                                                      |                | alumina  | 3 mm            |                           |                             |          |         |
| Comparative                                                          | H              | alumina  | 3 mm            | —                         | 12% increase                | 0.0711   | 0.116   |
| Example 1                                                            |                |          |                 |                           |                             |          |         |
| Comparative                                                          | I              | zirconia | 3 mm            | 10 m/s                    | 8% increase                 | 0.0641   | 0.994   |
| Example 2                                                            |                |          |                 |                           |                             |          |         |
| Comparative                                                          | N              | —        | —               | —                         | 19% increase                | 0.08741  | 0.1009  |
| Example 5                                                            |                |          |                 |                           |                             |          |         |

—: Not applicable or not measured

TABLE 3

|                       | Coating liquid | Absorbance difference |
|-----------------------|----------------|-----------------------|
| Example 2             | B              | 0.69                  |
| Example 5             | E              | 0.98                  |
| Example 6             | F              | 0.92                  |
| Example 7             | G              | 0.014                 |
| Comparative Example 1 | H              | 1.649                 |
| Comparative Example 3 | J              | 1.076                 |
| Comparative Example 4 | K              | 1.957                 |
| Comparative Example 5 | N              | 0.056                 |

25 containing particles having an average diameter of 0.10 μm or less highly affect the characteristics of the mixture.

## Example 10

The coating liquid A for forming an undercoat layer was applied to a cut aluminum tube having an outer diameter of 24 mm, a length of 236.5 mm, and a thickness of 0.75 mm by dipping to form an undercoat layer with a dried thickness of 2 μm. The surface of the undercoat layer was observed by a scanning electron microscope to confirm substantially no agglomeration.

TABLE 4

| Regular reflection rate (%) of undercoat layer |                |                        |                              |                              |                               |
|------------------------------------------------|----------------|------------------------|------------------------------|------------------------------|-------------------------------|
|                                                | Coating liquid | Measurement wavelength | Extruded mirror surface tube | Cut tube (cut pitch: 0.6 mm) | Cut tube (cut pitch: 0.95 mm) |
| Example 2                                      | B              | 480 nm                 | 57.4                         | 57.3                         | 57.8                          |
| Example 5                                      | E              | 480 nm                 | 56.7                         | 56.4                         | 54.9                          |
| Example 6                                      | F              | 480 nm                 | 57.6                         | 56.5                         | 58.6                          |
| Example 7                                      | G              | 400 nm                 | 64.6                         | 65.4                         | 57.2                          |
| Comparative                                    | H              | 480 nm                 | 40.2                         | 39.8                         | 41.8                          |
| Example 1                                      |                |                        |                              |                              |                               |
| Comparative                                    | J              | 480 nm                 | 35.8                         | 37.1                         | 37.5                          |
| Example 3                                      |                |                        |                              |                              |                               |
| Comparative                                    | K              | 480 nm                 | 26.2                         | 25.0                         | 27.5                          |
| Example 4                                      |                |                        |                              |                              |                               |
| Comparative                                    | N              | 400 nm                 | 48.3                         | 49.0                         | 39.6                          |
| Example 5                                      |                |                        |                              |                              |                               |

The coating liquids for forming an undercoat layer prepared by the process of the present invention have small average particle diameters and small particle size distribution widths, and consequently have high stability and are capable of forming a uniform undercoat layer. In addition, viscosity is not significantly increased even when stored for a long period of time, thus showing high stability. Furthermore, the undercoat layers formed with the coating liquids for forming an undercoat layer have high uniformity not to highly scatter light, thus exhibiting high regular reflection rates.

Furthermore, it was confirmed that, in a mixture of liquids containing particles having different average diameters, additivity is not observed and the characteristics of the liquid

55 A dispersion was prepared by mixing 20 parts by weight of oxytitanium phthalocyanine, as a charge-generating material, having a powder X-ray diffraction spectrum pattern to CuK $\alpha$  characteristic X-rays shown in FIG. 3 and 280 parts by weight of 1,2-dimethoxyethane and subjecting the mixture to dispersion treatment in a sand grind mill for 2 hours. Then, this dispersion was mixed with 10 parts by weight of polyvinyl butyral (trade name "Denka Butyral" #6000C, manufactured by Denki Kagaku Kogyo K.K.), 253 parts by weight of 1,2-dimethoxyethane, and 85 parts by weight of 4-methoxy-4-methylpentanone-2. The mixture was further mixed with 234 parts by weight of 1,2-dimethoxyethane, and the resulting mixture was treated with an ultrasonic dispersing device and then filtered through a PTFE membrane filter with a pore size

49

of 5  $\mu\text{m}$  (Mitex LC, manufactured by Advantech Co., Ltd.) to give a coating liquid for forming a charge-generating layer. This coating liquid for forming a charge-generating layer was applied onto the undercoat layer by dipping and dried to form a charge-generating layer having a dried thickness of 0.4  $\mu\text{m}$ .

Then, on this charge-generating layer was applied a coating liquid for forming a charge-transporting layer prepared by dissolving 56 parts of a hydrazone compound shown below:

### [Chemical Formula 5]



14 parts of a hydrazone compound shown below:

### [Chemical Formula 6]



100 parts of a polycarbonate resin having a repeating structure shown below:

### [Chemical Formula 7]



and 0.05 part of a silicone oil in 640 parts by weight of a solvent mixture of tetrahydrofuran/toluene (8/2). By the air-drying at room temperature for 25 minutes, a layer with a thickness of 17  $\mu\text{m}$  was given. The layer was further dried at 125° C. for 20 minutes to form an electrophotographic photo-

50

photoreceptor having a charge-transporting layer. The thus prepared electrophotographic photoreceptor was used as photoreceptor P1.

The dielectric breakdown strength of the photoreceptor P1 was measured as follows: The photoreceptor was fixed at a temperature of 25° C. and a relative humidity of 50%, and a charging roller having a volume resistivity of about  $2 \text{ M}\Omega\cdot\text{cm}$  and having a length about 2 cm shorter than that of the drum at both ends was pressed on the photoreceptor for applying a direct-current voltage of -3 kV, and the time until dielectric breakdown was measured. The results are shown in Table 5.

The photoreceptor was mounted on an electrophotographic characteristic evaluation device produced in accordance with a standard of The Society of Electrophotography of Japan (Densi Shashin Gifyutsu no Kiso to Oyo Zoku (Fundamentals and Applications of Electrophotography II) edited by The Society of Electrophotography of Japan, published by Corona Publishing Co., Ltd., pp. 404-405) and was charged such that the surface potential was -700 V and then was irradiated with a 780 nm laser at an intensity of  $5.0 \mu\text{J}/\text{cm}^2$ . The surface potential at 100 ms after the exposure was measured at  $25^\circ \text{C}$ . and a relative humidity of 50% (hereinafter, optionally, referred to as NN circumstances) and at  $5^\circ \text{C}$ . and a relative humidity of 10% (hereinafter, optionally, referred to as LL circumstances). The results are shown in Table 5.

### Example 11

A photoreceptor P2 was produced as in Example 10 except that the thickness of the undercoat layer was 3  $\mu\text{m}$ . The surface of the undercoat layer was observed with a scanning electron microscope as in Example 10 to confirm substantially no agglomeration. The photoreceptor P2 was evaluated as in Example 10. The results are shown in Table 5.

### Example 12

A coating liquid **A2** for forming an undercoat layer was prepared as in Example 1 except that the weight ratio of titanium oxide and a copolymerized polyamide (titanium oxide/copolymerized polyamide) was 2/1.

45 A photoreceptor P3 was produced as in Example 10 except that the coating liquid A2 was used as a coating liquid for

65 forming an undercoat layer. The surface of the undercoat layer was observed with a scanning electron microscope as in Example 10 to confirm substantially no agglomeration. The photoreceptor P3 was evaluated as in Example 10. The results are shown in Table 5.

51

## Example 13

A photoreceptor Q1 was produced as in Example 10 except that the coating liquid B for forming an undercoat layer described in Example 2 was used as a coating liquid for forming an undercoat layer. The surface of the undercoat layer was observed with a scanning electron microscope as in Example 10 to confirm substantially no agglomeration. The surface state of the undercoat layer was measured with Micro-map manufactured by Ryoka Systems Inc. in a Wave mode, at a measurement wavelength of 552 nm, at a magnification of objective lens of 40 times, with a measurement area of 190  $\mu\text{m}$  by 148  $\mu\text{m}$ , and with background shape correction (Term) of cylinder. The in-plane root mean square roughness (RMS) was 43.2 nm, the in-plane arithmetic mean roughness (Ra) was 30.7 nm, and the in-plane maximum roughness (P-V) was 744 nm. The photoreceptor Q1 was evaluated as in Example 10. The results are shown in Table 5.

## Example 14

A photoreceptor Q2 was produced as in Example 13 except that the thickness of the undercoat layer was 3  $\mu\text{m}$ . The surface of the undercoat layer was observed with a scanning electron microscope as in Example 10 to confirm substantially no agglomeration. The photoreceptor Q2 was evaluated as in Example 10. The results are shown in Table 5.

## Example 15

A photoreceptor Q3 was produced as in Example 13 except that the coating liquid E was used as a coating liquid for forming an undercoat layer. The surface of the undercoat layer was observed with a scanning electron microscope as in Example 10 to confirm substantially no agglomeration. The photoreceptor Q3 was evaluated as in Example 10. The results are shown in Table 5.

## Example 16

A photoreceptor R1 was produced as in Example 10 except that the coating liquid C for forming an undercoat layer described in Example 3 was used as a coating liquid for forming an undercoat layer. The surface of the undercoat layer was observed with a scanning electron microscope as in Example 10 to confirm substantially no agglomeration. The photoreceptor R1 was evaluated as in Example 10. The results are shown in Table 5.

## Example 17

A photoreceptor R2 was produced as in Example 16 except that the thickness of the undercoat layer was 3  $\mu\text{m}$ . The surface of the undercoat layer was observed with a scanning electron microscope as in Example 10 to confirm substantially no agglomeration. The photoreceptor R2 was evaluated as in Example 10. The results are shown in Table 5.

## Example 18

A coating liquid C2 for forming an undercoat layer was prepared as in Example 3 except that the weight ratio of titanium oxide and a copolymerized polyamide (titanium oxide/copolymerized polyamide) was 2/1.

A photoreceptor R3 was produced as in Example 16 except that the coating liquid C2 was used as a coating liquid for forming an undercoat layer. The surface of the undercoat layer was observed with a scanning electron microscope as in Example 10 to confirm substantially no agglomeration. The photoreceptor R3 was evaluated as in Example 10. The results are shown in Table 5.

## Example 19

A photoreceptor S1 was produced as in Example 10 except that the coating liquid D for forming an undercoat layer described in Example 4 was used as a coating liquid for forming an undercoat layer. The surface of the undercoat layer was observed with a scanning electron microscope as in

52

Example 10 to confirm substantially no agglomeration. The surface state of the undercoat layer was measured as in Example 10. The in-plane root mean square roughness (RMS) was 25.5 nm, the in-plane arithmetic mean roughness (Ra) was 17.7 nm, and the in-plane maximum roughness (P-V) was 510 nm. The photoreceptor S1 was evaluated as in Example 10. The results are shown in Table 5.

## Example 20

A photoreceptor S2 was produced as in Example 19 except that the thickness of the undercoat layer was 3  $\mu\text{m}$ . The surface of the undercoat layer was observed with a scanning electron microscope as in Example 10 to confirm substantially no agglomeration. The photoreceptor S2 was evaluated as in Example 10. The results are shown in Table 5.

## Example 21

A coating liquid D2 for forming an undercoat layer was prepared as in Example 4 except that the weight ratio of titanium oxide and a copolymerized polyamide (titanium oxide/copolymerized polyamide) was 2/1.

A photoreceptor S3 was produced as in Example 19 except that the coating liquid D2 was used as a coating liquid for forming an undercoat layer. The surface of the undercoat layer was observed with a scanning electron microscope as in Example 10 to confirm substantially no agglomeration. The photoreceptor S3 was evaluated as in Example 10. The results are shown in Table 5.

## Comparative Example 6

A photoreceptor T1 was produced as in Example 10 except that the coating liquid H for forming an undercoat layer described in Comparative Example 1 was used as a coating liquid for forming an undercoat layer. The surface of the undercoat layer was observed with a scanning electron microscope as in Example 10 to confirm a large number of titanium oxide agglomerations. The surface state of the undercoat layer was measured as in Example 13. The in-plane root mean square roughness (RMS) was 148.4 nm, the in-plane arithmetic mean roughness (Ra) was 95.3 nm, and the in-plane maximum roughness (P-V) was 2565 nm. The photoreceptor T1 was evaluated as in Example 10. The results are shown in Table 5.

## Comparative Example 7

A photoreceptor T2 was produced as in Comparative Example 6 except that the thickness of the undercoat layer was 3  $\mu\text{m}$ . The surface of the undercoat layer was observed with a scanning electron microscope as in Example 10 to confirm a large number of titanium oxide agglomerations. The photoreceptor T2 was evaluated as in Example 10. The results are shown in Table 5.

## Comparative Example 8

A photoreceptor T3 was produced as in Comparative Example 6 except that the coating liquid J was used as a coating liquid for forming an undercoat layer. The surface of the undercoat layer was observed with a scanning electron microscope as in Example 10 to confirm a large number of titanium oxide agglomerations. The photoreceptor T3 was evaluated as in Example 10. The results are shown in Table 5.

## Comparative Example 9

A photoreceptor U1 was produced as in Example 10 except that the coating liquid I for forming an undercoat layer described in Comparative Example 2 was used as a coating liquid for forming an undercoat layer. The surface of the undercoat layer was observed with a scanning electron microscope as in Example 10 to confirm a large number of titanium oxide agglomerations. In the undercoat layer of the photoreceptor U1, the components were inhomogeneous and the thickness was uneven. Consequently, the electric characteristics were not evaluated.

TABLE 5

| Electric characteristics of photoreceptor and time until dielectric breakdown |                                                       |     |           |         |                                 |          |
|-------------------------------------------------------------------------------|-------------------------------------------------------|-----|-----------|---------|---------------------------------|----------|
| Photoreceptor                                                                 | Titanium oxide/copolymerized polyamide (weight ratio) |     | Undercoat |         | Time until dielectric breakdown |          |
|                                                                               | VL (NN)                                               | LL  | VL        | VL (NN) | LL                              |          |
| Example 10                                                                    | P1                                                    | 3/1 | 2 μm      | -77 V   | -175 V                          | 20.5 min |
| Example 11                                                                    | P2                                                    | 3/1 | 3 μm      | —       | —                               | —        |
| Example 12                                                                    | P3                                                    | 2/1 | 2 μm      | -98 V   | -221 V                          | 21.8 min |
| Example 13                                                                    | Q1                                                    | 3/1 | 2 μm      | -77 V   | -174 V                          | 18.5 min |
| Example 14                                                                    | Q2                                                    | 3/1 | 3 μm      | -82 V   | -195 V                          | —        |
| Example 15                                                                    | Q3                                                    | 2/1 | 2 μm      | -98 V   | -223 V                          | 21.4 min |
| Example 16                                                                    | R1                                                    | 3/1 | 2 μm      | -77 V   | -161 V                          | 16.1 min |
| Example 17                                                                    | R2                                                    | 3/1 | 3 μm      | -81 V   | -176 V                          | —        |
| Example 18                                                                    | R3                                                    | 2/1 | 2 μm      | -102 V  | -218 V                          | 20.2 min |
| Example 19                                                                    | S1                                                    | 3/1 | 2 μm      | -83 V   | -176 V                          | 13.6 min |
| Example 20                                                                    | S2                                                    | 3/1 | 3 μm      | -87 V   | -191 V                          | —        |
| Example 21                                                                    | S3                                                    | 2/1 | 2 μm      | -109 V  | -232 V                          | 21.4 min |
| Comparative                                                                   | T1                                                    | 3/1 | 2 μm      | -76 V   | -151 V                          | 2.8 min  |
| Example 6                                                                     |                                                       |     |           |         |                                 |          |
| Comparative                                                                   | T2                                                    | 3/1 | 3 μm      | -82 V   | -175 V                          | —        |
| Example 7                                                                     |                                                       |     |           |         |                                 |          |
| Comparative                                                                   | T3                                                    | 2/1 | 2 μm      | -103 V  | -215 V                          | 14.6 min |
| Example 8                                                                     |                                                       |     |           |         |                                 |          |
| Comparative                                                                   | U1                                                    | 3/1 | 2 μm      |         |                                 |          |
| Example 9                                                                     |                                                       |     |           |         |                                 |          |

35

The electrophotographic photoreceptors of the present invention had homogeneous undercoat layers without agglomeration and exhibited low potential variation due to environmental variation and high resistance to dielectric breakdown.

### Example 22

The coating liquid B for forming an undercoat layer, which was prepared in Example 2 (sic), was applied to a cut aluminum tube with an outer diameter of 30 mm, a length of 285 mm, and a thickness of 0.8 mm by dipping to form an under-

coat layer with a dried thickness of 2.4  $\mu\text{m}$ . The surface of the undercoat layer was observed with a scanning electron microscope to confirm substantially no agglomeration.

40 A coating liquid for forming a charge-generating layer was prepared as in Example 10 and was applied onto the under-coat layer by dipping to form a charge-generating layer having a dried thickness of 2.4  $\mu\text{m}$ .

Then, on this charge-generating layer was applied a coating liquid containing 60 parts of a composition (A) described in Example 1 of Japanese Unexamined Patent Application Publication No. 2002-080432 as a charge-transporting material having the following main structure:

### [Chemical Formula 8]

### composition (A)



100 parts of a polycarbonate resin having a repeating structure shown below:

[Chemical Formula 9]



8 parts of BHT, and 0.05 part by weight of a silicone oil in 640 parts by weight of a solvent mixture of tetrahydrofuran/toluene (8/2) to give a charge-transporting layer with a dried thickness of 10  $\mu\text{m}$ . The layer was further dried to form an electrophotographic photoreceptor having the charge-transporting layer.

The produced photoreceptor was mounted on a cartridge (having a scorotron charging member and a blade cleaning member as an imaging unit cartridge) of a color printer (product name: InterColor LP-1500C, manufactured by Seiko Epson Corp.) to form a full-color image. The printed image was satisfactory. The number of small color spots observed in 1.6 cm square in the image is shown in Table 6.

The resulting photoreceptor (one week after the production) was rotated at a predetermined velocity using an electrophotographic characteristic evaluation device produced in accordance with a standard of The Society of Electrophotography of Japan (Densi Shashin Gizyutsu no Kiso to Oyo Zoku (Fundamentals and Applications of Electrophotography II) edited by The Society of Electrophotography of Japan, published by Corona Publishing Co., Ltd., pp. 404-405), and electric characteristics of the photoreceptor were evaluated for the cycle of charging, exposure, potential measurement, and charge elimination. The evaluation was performed at an initial surface potential of -700 V using monochromatic light of 780 nm for exposure and 660 nm for charge elimination. As an indicator of sensitivity, the exposure energy (half-decay exposure energy) required for the surface potential to reach -350 V was measured at 25° C. and a relative humidity of 50%. A decrease in surface potential (DD) from the initial surface potential (-700 V) when left in a dark place for 5 seconds was measured. The results are shown in Table 6.

#### Example 23

A full-color image was formed as in Example 22 except that the coating liquid 3AH for forming an undercoat layer was used as a coating liquid for forming an undercoat layer. The printed image was satisfactory. The number of small color spots observed in 1.6 cm square in the image is shown in Table 6. The electrophotographic characteristics were measured as in Example 22. The results are shown in Table 6.

#### Example 24

A full-color image was formed as in Example 22 except that the coating liquid AH for forming an undercoat layer was used as a coating liquid for forming an undercoat layer. The printed image was satisfactory. The number of small color spots observed in 1.6 cm square in the image is shown in Table 6. The electrophotographic characteristics were measured as in Example 22. The results are shown in Table 6.

#### Example 25

A full-color image was formed as in Example 22 except that the coating liquid A3H for forming an undercoat layer

was used as a coating liquid for forming an undercoat layer. The printed image was satisfactory. The number of small

color spots observed in 1.6 cm square in the image is shown in Table 6. The electrophotographic characteristics were measured as in Example 22. The results are shown in Table 6.

#### Comparative Example 10

An electrophotographic photoreceptor was produced as in Example 22 except that the coating liquid H for forming an undercoat layer described in Comparative Example 1 was used as a coating liquid for forming an undercoat layer.

A full-color image was formed using this electrophotographic photoreceptor. The printed image had a large number of color spots and was thus unsatisfactory. The number of the small color spots observed in 1.6 cm square in the image is shown in Table 6. The electrophotographic characteristics were measured as in Example 22. The results are shown in Table 6.

TABLE 6

|                        | Number of small color spot | Half-decay exposure energy ( $\mu\text{J}/\text{cm}^2$ ) | DD (%) |
|------------------------|----------------------------|----------------------------------------------------------|--------|
| Example 22             | 3                          | 0.182                                                    | 6.0    |
| Example 23             | 5                          | 0.182                                                    | 6.7    |
| Example 24             | 5                          | 0.183                                                    | 6.6    |
| Example 25             | 8                          | 0.182                                                    | 6.9    |
| Comparative Example 10 | 28                         | 0.182                                                    | 15.3   |

The electrophotographic photoreceptors of the present invention had excellent photoreceptive characteristics and high resistance to dielectric breakdown and also had significantly excellent performances, i.e., reduced image defects such as color spots.

The photoreceptor produced in Example 22 was fixed at 25° C. and a relative humidity of 50%, and a charging roller having a volume resistivity of about 2  $\text{M}\Omega\cdot\text{cm}$  and having a length about 2 cm shorter than that of the drum at both ends was pressed on the photoreceptor. A current of 2.6  $\mu\text{A}$  flew when a direct-current voltage of -2 kV was applied to the photoreceptor. Then, the voltage applied was increased to -3 kV, but dielectric breakdown did not occur.

The photoreceptor produced in Example 23 was fixed at 25° C. and a relative humidity of 50%, and a charging roller having a volume resistivity of about 2  $\text{M}\Omega\cdot\text{cm}$  and having a length about 2 cm shorter than that of the drum at both ends was pressed on the photoreceptor. A current of 4.0  $\mu\text{A}$  flew when a direct-current voltage of -2 kV was applied to the photoreceptor. Then, the voltage applied was increased to -3 kV, but dielectric breakdown did not occur.

The photoreceptor produced in Example 24 was fixed at 25° C. and a relative humidity of 50%, and a charging roller having a volume resistivity of about 2  $\text{M}\Omega\cdot\text{cm}$  and having a length about 2 cm shorter than that of the drum at both ends was pressed on the photoreceptor. A current of 5.5  $\mu\text{A}$  flew when a direct-current voltage of -2 kV was applied to the

photoreceptor. Then, the voltage applied was increased to  $-3$  kV, but dielectric breakdown did not occur.

The photoreceptor produced in Example 25 was fixed at  $25^{\circ}\text{C}$ . and a relative humidity of 50%, and a charging roller having a volume resistivity of about  $2\text{ M}\Omega\cdot\text{cm}$  and having a length about 2 cm shorter than that of the drum at both ends was pressed on the photoreceptor. A current of  $7.1\text{ }\mu\text{A}$  flew when a direct-current voltage of  $-2\text{ kV}$  was applied to the photoreceptor. Then, the voltage applied was increased to  $-3\text{ kV}$ , but dielectric breakdown did not occur.

The photoreceptor produced in Example 25 was fixed at  $25^{\circ}\text{C}$ . and a relative humidity of 50%, and a charging roller having a volume resistivity of about  $2\text{ M}\Omega\cdot\text{cm}$  and having a length about 2 cm shorter than that of the drum at both ends was pressed on the photoreceptor. A current of  $22\text{ }\mu\text{A}$  flew when a direct-current voltage of  $-2\text{ kV}$  was applied to the photoreceptor. Then, dielectric breakdown occurred during the increase of the voltage to  $-3\text{ kV}$ .

#### Example 26

The photoreceptor Q1 produced in Example 13 was mounted on a printer ML1430 (including an integrated cartridge consisting of a contact-type charging roller member and a monochrome development member) manufactured by Samsung Co., Ltd., and image formation was repeated at a printing concentration of 5% for observing image defects due to dielectric breakdown. No image defect was observed in 50000 images formed.

#### Comparative Example 11

The photoreceptor T1 produced in Comparative Example 6 was mounted on a printer ML1430 manufactured by Samsung Co., Ltd. Image formation was repeated at a printing concentration of 5% for observing image defects caused by dielectric breakdown, and image defect was observed when 35000 images were formed.

#### Example 27

The coating liquid 3AH for forming an undercoat layer, which was prepared in Example 8A, was applied to a cut aluminum tube with an outer diameter of 24 mm, a length of 236.5 mm, and a thickness of 0.75 mm by dipping to form an undercoat layer with a dried thickness of  $2\text{ }\mu\text{m}$ .

After mixing 1.5 parts of a charge-generating material represented by the following Formula:

[Chemical Formula 10]



(where Z denotes a mixture of and )

and 30 parts of 1,2-dimethoxyethane, the material was pulverized in a sand grind mill for 8 hours for microparticle dispersion treatment. Then, the mixture was mixed with a binder liquid prepared by dissolving 0.75 part of polyvinyl butyral (trade name "Denka Butyral" #6000C, manufactured by Denki Kagaku Kogyo K.K.) and 0.75 part of a phenoxy resin (PKHH, a product of Union Carbide Corp.) in 28.5 parts of 1,2-dimethoxyethane. Finally, 13.5 parts of an arbitrary liquid mixture of 1,2-dimethoxyethane and 4-methoxy-4-methyl-2-pentanone was added to the mixture to prepare a coating liquid for forming a charge-generating layer containing 4.0 wt % solid components (pigment and resin). This coating liquid for forming a charge-generating layer was applied onto the undercoat layer by dipping and drying it to form a charge-generating layer having a dried thickness of  $0.6\text{ }\mu\text{m}$ .

Then, on this charge-generating layer applied was a coating liquid for forming a charge-transporting layer prepared by dissolving 67 parts of a triphenylamine compound shown below:

20

[Chemical Formula 11]



100 parts of a polycarbonate resin having a repeating structure shown below:

[Chemical Formula 12]



0.5 part of a compound having the following structure:

[Chemical Formula 13]



and 0.02 part by weight of a silicone oil in 640 parts by weight of a solvent mixture of tetrahydrofuran/toluene (8/2). The applied liquid was air-dried at room temperature for 25 minutes to give a charge-transporting layer with a dried thickness of 25  $\mu\text{m}$ . The layer was further dried at 125° C. for 20 minutes to form an electrophotographic photoreceptor having the charge-transporting layer.

The resulting electrophotographic photoreceptor was mounted on an electrophotographic characteristic evaluation device produced in accordance with a standard of The Society of Electrophotography of Japan (Densi Shashin Gizyutsu no Kiso to Oyo Zoku (Fundamentals and Applications of Electrophotography II) edited by The Society of Electrophotography of Japan, published by Corona Publishing Co., Ltd., pp. 404-405), and electric characteristics thereof were evaluated by the cycle of charging, exposure, potential measurement, and charge elimination, according to the following procedure.

The initial surface potential of the photoreceptor that was charged by discharging with a scorotron charging device at a grid voltage of -800 V in a dark place was measured. Then, the photoreceptor was irradiated with monochromatic light of 450 nm emitted from a halogen lamp and monochromatized through an interference filter. The irradiation energy ( $\mu\text{J}/\text{cm}^2$ ) required for the surface potential to reach -350 V was measured as sensitivity E1/2. The initial charging potential was -710 V, and the sensitivity E1/2 was 3.290  $\mu\text{J}/\text{cm}^2$ . A larger value of the initial charging potential (a larger absolute value of the potential) represents a better charging property, and a lower value of the sensitivity represents a higher sensitivity.

#### Comparative Example 12

An electrophotographic photoreceptor was produced as in Example 27 except that the coating liquid H for forming an undercoat layer described in Comparative Example 1 was used as a coating liquid for forming an undercoat layer. The electric characteristics of this electrophotographic photoreceptor were evaluated as in Example 27. The initial charging potential was -696 V and the sensitivity E1/2 was 3.304  $\mu\text{J}/\text{cm}^2$ .

The results in Example 27 and Comparative Example 12 elucidate that the electrophotographic photoreceptor of the present invention had high sensitivity to exposure to monochromatic light having a wavelength of 350 nm to 600 nm.

#### Industrial Applicability

The coating liquid for forming an undercoat layer of the present invention has high storage stability and enables to efficiently produce an electrophotographic photoreceptor with high quality by forming an undercoat layer of the photoreceptor by application of the coating liquid. The electrophotographic photoreceptor exhibits excellent duration stability and hardly causes image defects, and, consequently, an image-forming apparatus including the photoreceptor is capable of forming a high-quality image. Furthermore, according to the process for preparing the coating liquid, the coating liquid for forming an undercoat layer is efficiently prepared, and also the resulting coating liquid for forming an

undercoat layer has higher storage stability. Accordingly, the resulting electrophotographic photoreceptor has higher quality. Consequently, the present invention can be preferably applied to various fields where electrophotographic photoreceptors are used, for example, fields of copiers, printers, and printing machines.

The present invention can be applied to any industrial field, in particular, can be preferably applied to, for example, printers, facsimile machines, and copiers of electrophotographic systems.

10 Although the present invention has been described in detail with reference to certain preferred embodiments, those skilled in the art will recognize that various modifications will be made without departing from the purpose and scope of the present invention.

15 The present application is based on Japanese Patent Application (Patent Application No. 2006-140863) filed on May 19, 2006, the entire contents of which are hereby incorporated by reference.

20 The invention claimed is:

1. A coating liquid, comprising:  
metal oxide particles combined with a binder resin,  
wherein the metal oxide particles have a number average  
particle diameter ( $M_p$ ) of  $0 < M_p \leq 0.10 \mu\text{m}$  and a 10%  
cumulative particle diameter ( $D_{10}$ ) of  $0 < D_{10} \leq 0.060 \mu\text{m}$ ,  
in the coating liquid for forming an undercoat layer  
of an electrophotographic photoreceptor.

25 2. A process for preparing a coating liquid comprising:  
liquid metal oxide particles and a binder resin, comprising:  
dispersing the metal oxide particles with a medium having  
an average particle diameter of 5 to 200  $\mu\text{m}$  in a wet  
agitating ball mill, wherein the metal oxide particles  
have a number average particle diameter ( $M_p$ ) of  
 $0 < M_p \leq 0.10 \mu\text{m}$  and a 10% cumulative particle diameter  
 $(D_{10})$  of  $0 < D_{10} \leq 0.060 \mu\text{m}$  which are measured by a  
dynamic light-scattering method, to form the coating  
liquid for forming an undercoat layer for an electropho-  
tographic photoreceptor.

30 3. The process for preparing a coating liquid according to  
claim 2, wherein the wet agitating ball mill includes a stator,  
a slurry-supplying port disposed at one end of the stator, a  
slurry-discharging port disposed at the other end of the stator,  
a rotor for agitating and mixing the medium packed in the  
stator and slurry supplied from the supplying port, and a  
40 separator that is rotatably connected to the discharging port  
and separates the medium and the slurry by centrifugal force  
to discharge the slurry from the discharging port.

35 4. The process for preparing a coating liquid according to  
claim 3, wherein the separator of the wet agitating ball mill is  
connected to the discharging port to rotate in synchronization  
with the rotor and separates the medium and the slurry by the  
centrifugal force to discharge the slurry from the discharging  
port, and the separator is of an impeller-type including two  
50 disks having blade-fitting grooves on the inner faces facing  
each other, a blade fitted to the fitting grooves and lying  
between the disks, and supporting means which supports the  
disks having the blade therebetween from both sides.

5. A coating liquid for forming an undercoat layer prepared  
55 by the process according to claim 2.

6. An electrophotographic photoreceptor comprising an  
undercoat layer formed by applying and drying the coating  
liquid according to claim 1.

60 7. The electrophotographic photoreceptor according to  
claim 6, wherein the undercoat layer has a thickness of from  
0.1  $\mu\text{m}$  to 10  $\mu\text{m}$ , and wherein the electrophotographic pho-  
toreceptor is a multilayered photoreceptor of which one layer  
is a charge transporting layer that is formed of material having  
a thickness of from 5  $\mu\text{m}$  to 15  $\mu\text{m}$ .

65 8. An image-forming apparatus comprising an electropho-  
tographic photoreceptor, charging means for charging the  
electrophotographic photoreceptor, image exposure means  
for forming an electrostatic latent image by subjecting the

**61**

charged electrophotographic photoreceptor to image exposure, development means for developing the electrostatic latent image with toner, and transfer means for transferring the toner to a transfer object, wherein the photoreceptor is the electrophotographic photoreceptor according to claim 6.

9. The image-forming apparatus according to claim 8, wherein the charging means is in contact with the electrophotographic photoreceptor.

10. The image-forming apparatus according to claim 8, wherein the exposure light used in the image exposure means has a wavelength of from 350 nm to 600 nm.

11. An electrophotographic cartridge comprising an electrophotographic photoreceptor and at least one of a charging means for charging the electrophotographic photoreceptor and a development means for developing an electrostatic latent image formed in the photoreceptor with toner, wherein the photoreceptor is the electrophotographic photoreceptor according to claim 6.

12. The electrophotographic cartridge according to claim 11, wherein the charging means is arranged so as to be in contact with the electrophotographic photoreceptor.

13. An electrophotographic photoreceptor comprising an undercoat layer formed by applying and drying the coating liquid for forming an undercoating layer according to claim 5.

**62**

14. An image-forming apparatus comprising an electrophotographic photo-receptor, charging means for charging the electrophotographic photoreceptor, image exposure means for forming an electrostatic latent image by subjecting the charged electrophotographic photoreceptor to image exposure development means for developing the electrostatic latent image with toner, and transfer means for transferring the toner to a transfer object, wherein the photoreceptor is the electrophotographic photoreceptor according to claim 13.

15. An electrophotographic cartridge comprising an electrophotographic photoreceptor and at least one of charging means for charging the electrophotographic photoreceptor and development means for developing an electrostatic latent image formed on the photoreceptor with toner, wherein the photoreceptor is the electrophotographic photoreceptor according to claim 13.

16. The coating liquid of claim 1, wherein the metal oxide particles have a number average particle diameter of from 0.02 to 0.10  $\mu\text{m}$ , and a 10% cumulative particle diameter of from 0.01 to 0.060  $\mu\text{m}$ .

17. The coating liquid of claim 1, wherein the particle diameters are measured by a dynamic light-scattering method.

\* \* \* \* \*